



US006969435B1

(12) **United States Patent**  
**Hinshaw et al.**

(10) **Patent No.:** **US 6,969,435 B1**  
(45) **Date of Patent:** **\*Nov. 29, 2005**

(54) **METAL COMPLEXES FOR USE AS GAS GENERANTS**

(75) Inventors: **Jerald C. Hinshaw**, Farr West, UT (US); **Daniel W. Doll**, North Ogden, UT (US); **Reed J. Blau**, Richmond, UT (US); **Gary K. Lund**, Malad, ID (US)

(73) Assignee: **Alliant Techsystems Inc.**, Edina, MN (US)

(\*) Notice: Subject to any disclaimer, the term of this patent is extended or adjusted under 35 U.S.C. 154(b) by 0 days.

This patent is subject to a terminal disclaimer.

(21) Appl. No.: **09/025,345**

(22) Filed: **Feb. 18, 1998**

**Related U.S. Application Data**

(63) Continuation of application No. 08/507,552, filed on Jul. 26, 1995, now Pat. No. 5,725,699, which is a continuation-in-part of application No. 08/184,456, filed on Jan. 19, 1994, now abandoned.

(51) **Int. Cl.** <sup>7</sup> **C06B 31/00**

(52) **U.S. Cl.** **149/45**

(58) **Field of Search** **149/45**

(56) **References Cited**

**U.S. PATENT DOCUMENTS**

|             |           |                                |
|-------------|-----------|--------------------------------|
| 147,871 A   | 2/1874    | Shaw                           |
| 1,399,954 A | 12/1921   | Fulton                         |
| 2,220,891 A | * 11/1940 | Cook et al. .... 149/2         |
| 2,483,803 A | 10/1949   | Bridgeman et al.               |
| 2,981,616 A | 4/1961    | Boyer                          |
| 3,010,815 A | 11/1961   | Pierce et al.                  |
| 3,066,130 A | 11/1962   | Zhivadinovich et al.           |
| 3,066,139 A | 11/1962   | Zhivadinovich                  |
| 3,122,462 A | 2/1964    | Kaufman                        |
| 3,138,498 A | * 6/1964  | Rausch .... 149/36             |
| 3,405,068 A | 10/1968   | Hiltz                          |
| 3,447,955 A | 6/1969    | Wittenwyler et al.             |
| 3,450,414 A | 6/1969    | Kobori                         |
| 3,463,684 A | 8/1969    | Dehn                           |
| 3,664,898 A | 5/1972    | Taylor et al.                  |
| 3,673,015 A | 6/1972    | Sollott et al.                 |
| 3,674,059 A | 7/1972    | Stephenson                     |
| 3,692,495 A | * 9/1972  | Schneiter et al. .... 149/19.5 |
| 3,711,115 A | 1/1973    | Lohr                           |
| 3,723,205 A | 3/1973    | Scheffee                       |
| 3,741,585 A | 6/1973    | Hendrickson et al.             |
| 3,755,182 A | 8/1973    | Marshall                       |
| 3,773,351 A | 11/1973   | Catanzarite                    |
| 3,773,352 A | 11/1973   | Radke                          |
| 3,773,947 A | 11/1973   | Boyars et al.                  |
| 3,779,823 A | 12/1973   | Price et al.                   |
| 3,785,149 A | 1/1974    | Timmerman                      |
| 3,787,074 A | 1/1974    | Lewis et al.                   |
| 3,791,302 A | 2/1974    | McLeod                         |
| 3,797,854 A | * 3/1974  | Poole et al. .... 280/741      |
| 3,806,461 A | 4/1974    | Hendrickson et al.             |
| 3,810,655 A | 5/1974    | Pracher                        |

|             |           |                               |
|-------------|-----------|-------------------------------|
| 3,814,694 A | 6/1974    | Klager                        |
| 3,827,715 A | 8/1974    | Lynch                         |
| 3,833,029 A | 9/1974    | Munn                          |
| 3,833,432 A | 9/1974    | Moy et al.                    |
| 3,837,942 A | 9/1974    | Catanzarite                   |
| 3,862,866 A | 1/1975    | Timmerman et al.              |
| 3,868,124 A | 2/1975    | Johnson                       |
| 3,880,447 A | 4/1975    | Thom et al.                   |
| 3,880,595 A | 4/1975    | Timmerman                     |
| 3,883,373 A | 5/1975    | Sidebottom                    |
| 3,895,098 A | 7/1975    | Pietz                         |
| 3,897,235 A | 7/1975    | Hamilton et al.               |
| 3,901,747 A | 8/1975    | Garner                        |
| 3,902,934 A | 9/1975    | Timmerman                     |
| 3,910,805 A | 10/1975   | Catanzarite                   |
| 3,912,458 A | 10/1975   | Fukuma et al.                 |
| 3,912,561 A | 10/1975   | Doin et al.                   |
| 3,912,562 A | 10/1975   | Garner                        |
| 3,920,575 A | 11/1975   | Shiki                         |
| 3,921,497 A | * 11/1975 | Christmann et al. .... 102/23 |
| 3,931,040 A | 1/1976    | Breazeale                     |
| 3,933,543 A | 1/1976    | Madden                        |
| 3,934,984 A | 1/1976    | Marlow et al.                 |
| 3,936,330 A | 2/1976    | Dergazarian et al.            |
| 3,947,300 A | 3/1976    | Passauer et al.               |
| 3,950,009 A | 4/1976    | Hamilton                      |
| 3,964,255 A | 6/1976    | Catanzarite                   |
| 3,971,729 A | 7/1976    | Timmerman                     |
| 3,977,981 A | 8/1976    | Dunlop et al.                 |
| 3,986,908 A | 10/1976   | Grebert et al.                |
| 3,996,079 A | 12/1976   | DiValentin                    |
| 4,021,275 A | 5/1977    | Kishi et al.                  |
| 4,053,567 A | 10/1977   | Franz                         |
| 4,062,708 A | 12/1977   | Goetz                         |

(Continued)

**FOREIGN PATENT DOCUMENTS**

|    |              |         |
|----|--------------|---------|
| EP | 0 519 485 A1 | 12/1992 |
| EP | 0 716 060    | 6/1996  |
| WO | WO 95/04015  | 2/1995  |
| WO | WO 95/19944  | 7/1995  |

**OTHER PUBLICATIONS**

Bailar, J.C., Jr., et al., ed., *Inorganic Syntheses*, vol. 4, pp. 171-172 (1953).

(Continued)

*Primary Examiner*—Aileen Felton  
*(74) Attorney, Agent, or Firm*—TraskBritt

(57) **ABSTRACT**

Gas generating compositions and methods for their use are provided. Metal complexes are used as gas-generating compositions. These complexes are comprised of a metal cation template, a neutral ligand containing hydrogen and nitrogen, and sufficient oxidizing anion to balance the charge of the complex. The complexes are formulated such that when the complex combusts, nitrogen gas and water vapor is produced. Specific examples of such complexes include metal nitrite ammine, metal nitrate ammine, and metal perchlorate ammine complexes, as well as hydrazine complexes. A binder and co-oxidizer can be combined with the metal complexes to improve crush strength of the gas-generating compositions and to permit efficient combustion of the binder. Such gas-generating compositions are adaptable for use in gas-generating devices, such as automobile air bags.

**33 Claims, No Drawings**

## U.S. PATENT DOCUMENTS

|             |         |                        |               |          |                        |           |               |
|-------------|---------|------------------------|---------------|----------|------------------------|-----------|---------------|
| 4,114,591 A | 9/1978  | Nakagawa               | 5,019,192 A   | 5/1991   | Ramaswamy              |           |               |
| 4,115,999 A | *       | 9/1978                 | Diebold ..... | 149/19.4 | 5,019,220 A            | 5/1991    | Taylor et al. |
| 4,124,515 A | 11/1978 | Gruner et al.          | 5,022,674 A   | 6/1991   | Frantom et al.         |           |               |
| 4,128,996 A | 12/1978 | Garner et al.          | 5,024,160 A   | 6/1991   | Canterberry et al.     |           |               |
| 4,152,891 A | 5/1979  | Garner                 | 5,031,932 A   | 7/1991   | Frantom et al.         |           |               |
| 4,157,648 A | 6/1979  | Brennan et al.         | 5,033,390 A   | 7/1991   | Minert et al.          |           |               |
| 4,179,327 A | 12/1979 | Seldner                | 5,035,757 A   | 7/1991   | Poole                  |           |               |
| 4,185,008 A | 1/1980  | Caspari et al.         | 5,043,030 A   | 8/1991   | Ramaswamy              |           |               |
| 4,200,615 A | 4/1980  | Hamilton et al.        | 5,046,429 A   | 9/1991   | Swann et al.           |           |               |
| 4,203,786 A | 5/1980  | Garner                 | 5,052,817 A   | 10/1991  | Bement et al.          |           |               |
| 4,203,787 A | 5/1980  | Kirchoff et al.        | 5,060,973 A   | 10/1991  | Giovanetti             |           |               |
| 4,214,438 A | 7/1980  | Hamilton et al.        | 5,062,365 A   | 11/1991  | Canterberry            |           |               |
| 4,238,253 A | 12/1980 | Garner                 | 5,062,367 A   | 11/1991  | Hayashi et al.         |           |               |
| 4,244,758 A | 1/1981  | Garner et al.          | 5,071,630 A   | *        | Oberth .....           | 423/266   |               |
| 4,246,051 A | 1/1981  | Garner et al.          | 5,073,273 A   | 12/1991  | Gupta et al.           |           |               |
| 4,298,412 A | 11/1981 | Biddle et al.          | 5,074,940 A   | 12/1991  | Ochi et al.            |           |               |
| 4,306,499 A | 12/1981 | Holmes                 | 5,089,069 A   | 2/1992   | Ramaswamy et al.       |           |               |
| 4,336,085 A | 6/1982  | Walker et al.          | 5,094,475 A   | 3/1992   | Olsson et al.          |           |               |
| 4,337,102 A | 6/1982  | Oberth et al.          | 5,098,597 A   | 3/1992   | Rothgery et al.        |           |               |
| 4,339,288 A | 7/1982  | Camp                   | 5,100,172 A   | 3/1992   | Vanvoorhies et al.     |           |               |
| 4,369,079 A | 1/1983  | Shaw                   | 5,100,174 A   | 3/1992   | Jasken et al.          |           |               |
| 4,370,181 A | 1/1983  | Lundstrom et al.       | 5,104,466 A   | 4/1992   | Allard et al.          |           |               |
| 4,370,930 A | 2/1983  | Strasser et al.        | 5,125,684 A   | 6/1992   | Cartwright             |           |               |
| 4,376,002 A | 3/1983  | Utracki                | 5,141,734 A   | 8/1992   | Misra                  |           |               |
| 4,390,380 A | 6/1983  | Camp                   | 5,160,386 A   | 11/1992  | Lund et al.            |           |               |
| 4,407,119 A | 10/1983 | Biddle et al.          | 5,197,758 A   | *        | Lund et al. .....      | 149/61    |               |
| 4,414,902 A | 11/1983 | Strasser et al.        | 5,198,046 A   | 3/1993   | Bucerius et al.        |           |               |
| 4,424,086 A | 1/1984  | Christopher            | 5,212,343 A   | 5/1993   | Brupacher et al.       |           |               |
| 4,484,960 A | 11/1984 | Rucker                 | 5,263,740 A   | *        | Frey et al. .....      | 280/741   |               |
| 4,533,416 A | 8/1985  | Poole                  | 5,266,132 A   | 11/1993  | Danen et al.           |           |               |
| 4,547,235 A | 10/1985 | Schneiter et al.       | 5,320,382 A   | *        | Goldstein et al. ..... | 280/735   |               |
| 4,547,342 A | 10/1985 | Adams et al.           | 5,429,691 A   | 7/1995   | Hinshaw et al.         |           |               |
| 4,578,247 A | 3/1986  | Bolieau                | 5,439,537 A   | *        | Hinshaw et al. .....   | 149/37    |               |
| 4,590,860 A | 5/1986  | Kromrey                | 5,472,534 A   | *        | Wardle et al. .....    | 149/36    |               |
| 4,604,151 A | 8/1986  | Knowlton et al.        | 5,472,535 A   | 12/1995  | Mendenhall et al.      |           |               |
| 4,632,714 A | 12/1986 | Abegg et al.           | 5,501,823 A   | *        | Lund et al. .....      | 264/3.1   |               |
| 4,642,147 A | 2/1987  | Hyypa                  | 5,514,230 A   | 5/1996   | Khandhadia             |           |               |
| 4,664,033 A | 5/1987  | Burkdoll et al.        | 5,516,377 A   | 5/1996   | Highsmith et al.       |           |               |
| 4,690,063 A | 9/1987  | Granier et al.         | 5,531,473 A   | *        | Rink et al. .....      | 149/83    |               |
| 4,696,705 A | 9/1987  | Hamilton               | 5,531,941 A   | *        | Poole .....            | 264/3.4   |               |
| 4,698,107 A | 10/1987 | Goetz et al.           | 5,536,339 A   | 7/1996   | Verneker               |           |               |
| 4,699,400 A | 10/1987 | Adams et al.           | 5,538,568 A   | *        | Taylor et al. .....    | 149/70    |               |
| 4,734,141 A | 3/1988  | Cartwright et al.      | 5,542,704 A   | *        | Hamilton et al. .....  | 280/741   |               |
| H464 H      | 5/1988  | Lee et al.             | 5,545,272 A   | *        | Poole et al. .....     | 149/48    |               |
| 4,758,287 A | 7/1988  | Pietz                  | 5,589,141 A   | *        | Sides et al. .....     | 422/164   |               |
| 4,798,142 A | 1/1989  | Canterberry et al.     | 5,592,812 A   | 1/1997   | Hinshaw et al.         |           |               |
| 4,806,180 A | 2/1989  | Goetz et al.           | 5,608,183 A   | 3/1997   | Barnes et al.          |           |               |
| 4,833,996 A | 5/1989  | Hayashi et al.         | 5,635,668 A   | 6/1997   | Barnes et al.          |           |               |
| 4,834,817 A | 5/1989  | Zeuner et al.          | 5,663,524 A   | 9/1997   | Bucerius               |           |               |
| 4,834,818 A | 5/1989  | Kazumi et al.          | 5,673,935 A   | *        | Hinshaw et al. .....   | 149/45    |               |
| 4,865,667 A | 9/1989  | Zeuner et al.          | 5,677,510 A   | 10/1997  | Bucerius et al.        |           |               |
| 4,890,860 A | 1/1990  | Schneiter              | 5,725,699 A   | *        | Hinshaw et al. .....   | 149/45    |               |
| 4,907,509 A | 3/1990  | Lieberman              | 5,731,540 A   | *        | Flanigan et al. .....  | 149/109.6 |               |
| 4,909,549 A | 3/1990  | Poole et al.           | 5,880,595 A   | 3/1999   | Whetsel                |           |               |
| 4,919,897 A | 4/1990  | Bender et al.          | 6,039,820 A   | *        | Hinshaw et al. .....   | 149/45    |               |
| 4,925,600 A | *       | Hommel et al. .....    | 6,481,746 B1  | *        | Hinshaw et al. .....   | 280/741   |               |
| 4,931,111 A | 6/1990  | Poole et al.           | 149/109.6     | 11/2002  | Hinshaw et al. .....   | 420/164   |               |
| 4,931,112 A | 6/1990  | Wardle et al.          |               |          |                        |           |               |
| 4,948,439 A | 8/1990  | Poole et al.           |               |          |                        |           |               |
| 4,950,458 A | 8/1990  | Cunningham             |               |          |                        |           |               |
| 4,959,011 A | 9/1990  | Nilsson                |               |          |                        |           |               |
| 4,963,203 A | 10/1990 | Halcomb et al.         |               |          |                        |           |               |
| 4,981,534 A | 1/1991  | Scheffe                |               |          |                        |           |               |
| 4,982,664 A | 1/1991  | Norton                 |               |          |                        |           |               |
| 4,998,751 A | 3/1991  | Paxton et al.          |               |          |                        |           |               |
| 5,003,887 A | 4/1991  | Unterforsthuber et al. |               |          |                        |           |               |
| 5,004,586 A | 4/1991  | Hayashi et al.         |               |          |                        |           |               |
| 5,005,486 A | 4/1991  | Lenzen                 |               |          |                        |           |               |
| 5,015,309 A | 5/1991  | Wardle et al.          |               |          |                        |           |               |
| 5,015,311 A | 5/1991  | Ramaswamy              |               |          |                        |           |               |

## OTHER PUBLICATIONS

Huheey, J.E., Inorganic Chemistry, 3rd Ed., Harper & Row, pp. A-97-A-107 (1983).

Whitten, K.W., et al., General Chemistry, Saunders College Publishing, p. 167 (1981).

Frantom, Hybrid Airbag Inflator Technology, Airbag Int'l. Symposium on Sophisticated Car Occupant Safety Systems, Weinbrenner-Saal, Germany, Nov. 2-3, 1992.

Michael Laing, "mer- and fac-  $[\text{Co}(\text{NH}_3)_3 (\text{NO}_2)_3]$ : Do They Exist?", *Journal of Chemical Education*, vol. 62, No. 8, Aug. 1985, pp. 707-708.

- K. Wieghardt and H. Siebert, “ $\mu$ -Carboxylatodi- $\mu$ -Hydroxo-bis [triamminecobalt (III)] Complexes”, *Inorganic Synthesis*, 23, 1985, pp. 107–117.
- K.C. Patil, C. Nesamani, V.R. Pai Vemeker, “Synthesis and Characterisation of Metal Hydrazine Nitrate, Azide and Perchlorate Complexes”, *Synthesis and Reactivity in Inorganic and Metal Organic Chemistry*, 23(4), 1982, pp. 383–395.
- Von H. Siebert, “Isomere des Trinitrotriamminkobalt (III)”, *Z. Annorg. Allg. Chem.* 441, 1978, pp. 47–57.
- Shidlovskii, AA; Gorbunov, V.V.; Shmagin, L.F. (Mosk. Inst. Khim. Mashinostr., Moscow, USSR), “The combustion rates of  $[\text{Co}(\text{NH}_3)_6]$   $[\text{Co}(\text{NO}_2)_6]$  (I) [15742–33–3],  $[\text{Co}(\text{NH}_3)_3(\text{NO}_2)_3]$  (II) [13600–88–9],  $[\text{Co}(\text{NH}_3)_6](\text{NO}_2)_3$ , (III) [13841–86–6], and  $(\text{NH}_4)_3[\text{CO}(\text{NO}_6)]$  (IV) [14652–46–1] were studied at 10–100 atm. The heats of combustion of I, II, III, and IV were 693, 667, 380, and 345 cal/g; and the ignition temps. were 217, 220, 230, and 185. degree., resp. The combustion rates of I, II, and III increased with pressure and decreased in the order I>II>III. Compo. IV burned significantly more slowly and evolved brown fumes.” 87:70416 Study of Combustion of Nitrito–Ammonia complexes of cobalt (III). *Izv. Vyssh. Uchebn. Zabed., Khim., Tekhnol.*, 20(4), 610–12 (Russian) 1977. Coden: Ivukar.
- Robert B. Hagel and Leonard F. Druding, “The Triamine of Cobalt (III). I. Geometrical Isomers of Trinitrotriamminecobalt (III)”, *Inorganic Chemistry*, vol. 9, No. 6, Jun. 1970, pp. 1496–1503.
- N.G. Klyuchnikov and F.I. Para, “Preparation of Some Hydrazine Compounds of Palladium”, *Russian Journal of Inorganic Chemistry*, 13 (3), pp. 416–418.
- Muraji Shibata, Motoshichi Mori, and Eishin Kyuno “Synthesis of Nitroammine- and Cyanoamminecobalt (III) Complexes with Potassium Tricarbonatocobaltate (II) as Starting Material”, *Inorganic Chemistry*, vol. 3, No. 11, Nov. 1964, pp. 1573–1576.
- Gessner G. Hawley, “The Condensed Chemical Dictionary”, Van Nostrand Reinhold Company, 9th Edition, p. 227.
- Bailey et al., *Comprehensive Inorganic Chemistry*, vol. 3, pp. 60, 61, 170, 1249, 1250, 1266–1269, and 1366–1367 (1973).
- Ablov, A.V., et al., “Thermal decomposition of cobalt(III) ammines”, *Zhurnal Neorganicheskoi Khimii* (1969), *Chem. Abs.* 72:85795 (SciFinder).
- Anthavale, P.D., et al., “Catalytic activity of copper(II) ammine complexes supported on silica gel in the decomposition of hydrogen peroxide”, *Indian Journal of Technology* (1988), *Chem. Abs.*, 111:121746 (SciFinder).
- Beck, M.T., et al., “Reactions of the coordinated nitrite ions of nitroamminecobalt(III) complexes”, *Magyar Kemial Folyoirst* (1970), *Chem. Abs.* 72:128235 (SciFinder).
- Bhatta, D., et al., “Annealing of chemical radiation damage in hexammino- and nitratopentamminocobaltic nitrates”, *Indian Journal of Chemistry, Section A: Inorganic, Physical, Theoretical & Analytical* (1982), *Chem. Abs.* 98:63203 (SciFinder).
- Cotton, F. Albert, et al., *Advanced Inorganic Chemistry*, 5<sup>th</sup> Ed., John Wiley & Sons, New York, 1988, p. 363.
- Do Ngoc Hus, et al., “Spectrophotometric determination of the stability constants of ammine–nitrite–cobalt(II) complexes, with consideration of the effect of dissolved oxygen”, *Zhurnal Obshchei Khimii* (1988), *Chem. Abs.* 108:157228 (SciFinder).
- Fronczeck, F. R., et al., “Reinvestigation of the crystal structure of decaammine  $\mu$ -peroxodicobalt tetrathiocyanate,” *Acta Crystallographica, Section B: Structural Crystallography and Crystal Chemistry* (1974), *Chem. Abs.* 80:88249 (SciFinder).
- Hagel, R.B., et al., “The Triamines of Cobalt (III). I. Geometrical Isomers of Trinitrotriamminecobalt(III)”, *Inorganic Chemistry*, vol. 9, No. 6, Jun. 1970, pp. 1496–1502.
- Jackson, W.G., “Oxygen scrambling in pentaamminenitrocobalt(III) revisited”, *Inorganica Chimica Acta* (1988), *Chem. Abs.*, 109:177477 (SciFinder).
- Kapanadze, T. Sh., et al., “Cobalt(III) sulfito mixed ligand complexes”, *Koordinatsionnaya Khimiya* (1989), *Chem. Abs.*, 111:89270 (SciFinder).
- King, Henry C.A., “Solubilities and enthalpies of solution of a series of pentammine complexes”, *Revista Latinoamericana de Quimica* (1972), *Chem. Abs.* 76:158971 (SciFinder).
- King, H.J.S., “Researches on Chromammines, Part II, Hydroxopentamminochromic Salts and Electrical Conductivities of Chromammines”, *Hydroxopentamminochromic Salts, Etc.*, Jul. 1925, pp. 2100–2109.
- Klyuchnikov et al., “Conversion of Mononuclear Hydrazine Complexes of Platinum and Palladium into Bionuclear Complexes”, *Ukrainski f i Khimicheski f i Zhurnal*, vol. 36, No. 687, 1970, pp. 687–689.
- Klyuchnikov, N.G., et al., “Preparation of Some Hydrazine Compounds of Palladium”, *Russian Journal of Inorganic Chemistry*, 13 (3), 1968, pp. 416–418.
- Laing, M., “mer- and fac- $[\text{Co}(\text{NH}_3)_3(\text{NO}_2)_3]$ : Do They Exist?”, *Journal of Chemical Education*, vol. 62, No. 8, Aug. 1985, pp. 707–709.
- Marsh, R.E., et al., “Crystal structure of decammine- $\mu$ -peroxo-dicobalt pentanitrate”, *Acta Crystallographica, Section B: Structural Crystallography and Crystal Chemistry* (1968), *Chem. Abs.* 68:82052 (SciFinder).
- Miskowski, V. M., et al., “Crystal structure and polarized electronic spectra of a ( $\mu$ -peroxo)dicobalt(III) complex:  $[(\text{NH}_3)_5\text{Co}_2\text{O}_2](\text{NO}_3)_2\text{C}_13.2\text{H}_2\text{O}$ ”, *Inorganic Chemistry* (1984), *Chem. Abs.* 100:59011 (SciFinder).
- Mrozniski, J., “Thermal analysis of cobalt(III) peroxy complexes”, *Pol. Prace Naukowe Instytutu Chemii Nieorganicznej i Metalurgii Pierwiastkow Rzadkich Politechniki Wroclawskiej* (1973), *Chem. Abs.* 80:127685 (SciFinder).
- Nomiya, K., et al., “Synthesis of cobalt(III) molybdoheptopolyanions using carbonato–ammine cobalt(III) complexes as starting materials”, *Polyhedron* (1987), *Chem. Abs.* 107:189450 (SciFinder).
- Pass, G., et al., *Practical Inorganic Chemistry, Preparations, reactions and instrumental methods*, 2<sup>nd</sup> Ed., Chapter 6, *Coordination chemistry I: typical compounds*, Chapman and Hall, London, 1974, pp. 56–62.
- Patil, K.C., et al., “Synthesis and Characterisation of Metal Hydrazine Nitrate, Azide and Perchlorate Complexes”, *Synth. React. Inorg. Met.-Org. Chem.*, 12(4), 1982, pp. 383–395.
- Schmitz-Dumont, V.O., et al., “Hydroxokobalt(III)-amide”, *Z. anorg. allg. Chemie*, Bd. 300, 1959, pp. 175–193.
- Shibata, M., et al., “Synthesis of Nitroammine- and Cyanoamminecobalt(III) Complexes with Potassium Tricarbonatocobaltate(III) as the Starting Material”, *Inorganic Chemistry*, vol. 3, No. 11, Nov. 1964, pp. 1573–1576.

Shibata, M., "Optically active *cis*-unidentate-dicarbonato, *cis*-*cis*-diunidentate-carbonato, and unidentate glycinate cobalt(III) complexes," Inorganic Syntheses (1985), Chem. Abs. 104:121865 (SciFinder).  
Siebert, V.H., "Isomere des Trinitrotriamminkobalt(III)," Z. anorg. Allg. Chem. 441 (1978), pp. 47-57.  
Wieghardt, K., et al., " $\mu$ -Carboxylatodi- $\mu$ -Hydroxo-Bis [triamminecobalt(III)] Complexes," Inorganic Synthesis 23, 1985, pp. 107-116.

Mantell, C.L., The Water-Soluble Gums, Reinhold Publishing Corp., New York, 1947, pp. 19-46, 126-128, & 145-163.  
Patil, Proc.—Indian Acad. Sci., Chem. Sci (1986) 96(6), 459-64, abstract thereof, Chem. Abs., 106 #, 60349.  
Ellern, Military and Civilian Pyrotechnics, pp. 62-63 & 433, Chemical Publ. Company, Inc. (1986) New York.

\* cited by examiner

## METAL COMPLEXES FOR USE AS GAS GENERANTS

### RELATED APPLICATION

This invention is a continuation of application Ser. No. 08/507,552, filed Jul. 26, 1995, now U.S. Pat. No. 5,725,699, issued Mar. 10, 1998, which is a continuation-in-part of U.S. patent application Ser. No. 08/184,456, filed Jan. 19, 1994, titled "Metal Complexes For Use As Gas Generants," which is incorporated herein by reference, now abandoned.

### FIELD OF THE INVENTION

The present invention relates to complexes of transition metals or alkaline earth metals that are capable of combusting to generate gases. More particularly, the present invention relates to providing such complexes that rapidly oxidize to produce significant quantities of gases, particularly water vapor and nitrogen.

### BACKGROUND OF THE INVENTION

Gas-generating chemical compositions are useful in a number of different contexts. One important use for such compositions is in the operation of "air bags." Air bags are gaining in acceptance to the point that many, if not most, new automobiles are equipped with such devices. Indeed, many new automobiles are equipped with multiple air bags to protect the driver and passengers.

In the context of automobile air bags, sufficient gas must be generated to inflate the device within a fraction of a second. Between the time the car is impacted in an accident, and the time the driver would otherwise be thrust against the steering wheel, the air bag must fully inflate. As a consequence, nearly instantaneous gas generation is required.

There are a number of additional important design criteria that must be satisfied. Automobile manufacturers and others have set forth the required criteria that must be met in detailed specifications. Preparing gas-generating compositions that meet these important design criteria is an extremely difficult task. These specifications require that the gas-generating composition produce gas at a required rate. The specifications also place strict limits on the generation of toxic or harmful gases or solids. Examples of restricted gases include carbon monoxide, carbon dioxide,  $\text{NO}_x$ ,  $\text{SO}_x$ , and hydrogen sulfide.

The gas must be generated at a sufficiently and reasonably low temperature so that an occupant of the car is not burned upon impacting an inflated air bag. If the gas produced is overly hot, there is a possibility that the occupant of the motor vehicle may be burned upon impacting a just deployed air bag. Accordingly, it is necessary that the combination of the gas generant and the construction of the air bag isolates automobile occupants from excessive heat. All of this is required while the gas generant maintains an adequate-burn rate.

Another related but important design criteria is that the gas generant composition produces a limited quantity of particulate materials. Particulate materials can interfere with the operation of the supplemental restraint system, present an inhalation hazard, irritate the skin and eyes, or constitute a hazardous solid waste that must be dealt with after the operation of the safety device. In the absence of an acceptable alternative, the production of irritating particulates is one of the undesirable, but tolerated aspects of the currently used sodium azide materials.

In addition to producing limited, if any, quantities of particulates, it is desired that at least the bulk of any such particulates be easily filterable. For instance, it is desirable that the composition produce a filterable slag. If the reaction products form a filterable material, the products can be filtered and prevented from escaping into the surrounding environment.

Both organic and inorganic materials have been proposed as possible gas generants. Such gas generant compositions include oxidizers and fuels which react at sufficiently high rates to produce large quantities of gas in a fraction of a second.

At present, sodium azide is the most widely used and currently accepted gas-generating material. Sodium azide nominally meets industry specifications and guidelines. Nevertheless, sodium azide presents a number of persistent problems. Sodium azide is highly toxic as a starting material, since its toxicity level as measured by oral rat  $\text{LD}_{50}$  is in the range of 45 mg/kg. Workers who regularly handle sodium azide have experienced various health problems, such as severe headaches, shortness of breath, convulsions, and other symptoms.

In addition, no matter what auxiliary oxidizer is employed, the combustion products from a sodium azide gas generant include caustic reaction products such as sodium oxide, or sodium hydroxide. Molybdenum disulfide or sulfur have been used as an oxidizer for sodium azide. However, use of such oxidizers results in toxic products, such as hydrogen sulfide gas and corrosive materials such as sodium oxide and sodium sulfide. Rescue workers and automobile occupants have complained about both the hydrogen sulfide gas and the corrosive powder produced by the operation of sodium azide-based gas generants.

Increasing problems are also anticipated in relation to disposal of unused gas-inflated supplemental restraint systems, e.g., automobile air bags, in demolished cars. The sodium azide remaining in such supplemental restraint systems can leach out of the demolished car to become a water pollutant or toxic waste. Indeed, some have expressed concern that sodium azide might form explosive heavy metal azides or hydrazoic acid when contacted with battery acids following disposal.

Sodium azide-based gas generants are most commonly used for air bag inflation, but with the significant disadvantages of such compositions many alternative gas generant compositions have been proposed to replace sodium azide. Most of the proposed sodium azide replacements, however, fail to deal adequately with all of the criteria set forth above.

It will be appreciated, therefore, that there are a number of important criteria for selecting gas-generating compositions for use in automobile supplemental restraint systems. For example, it is important to select starting materials that are not toxic. At the same time, the combustion products must not be toxic or harmful. In this regard, industry standards limit the allowable amounts of various gases and particulates produced by the operation of supplemental restraint systems.

It would, therefore, be a significant advance to provide compositions capable of generating large quantities of gas that would overcome the problems identified in the existing art. It would be a further advance to provide a gas-generating composition that is based on substantially nontoxic starting materials and that produces substantially nontoxic reaction products. It would be another advance in the art to provide a gas-generating composition that produces very limited amounts of toxic or irritating particulate debris and limited

undesirable gaseous products. It would also be an advance to provide a gas-generating composition that forms a readily filterable solid slag upon reaction.

Such compositions and methods for their use are disclosed and claimed herein.

#### BRIEF SUMMARY OF THE INVENTION

The present invention is related to the use of complexes of transition metals or alkaline earth metals as gas-generating compositions. These complexes are comprised of a metal cation and a neutral ligand containing hydrogen and nitrogen. One or more oxidizing anions are provided to balance the charge of the complex. Examples of typical oxidizing anions that can be used include nitrates, nitrites, chlorates, perchlorates, peroxides, and superoxides. In some cases the oxidizing anion is part of the metal cation coordination complex. The complexes are formulated such that when the complex combusts, a mixture of gases containing nitrogen gas and water vapor are produced. A binder can be provided to improve the crush strength and other mechanical properties of the gas generant composition. A co-oxidizer can also be provided primarily to permit efficient combustion of the binder. Importantly, the production of undesirable gases or particulates is substantially reduced or eliminated.

Specific examples of the complexes used herein include metal nitrite ammines, metal nitrate ammines, metal perchlorate ammines, metal nitrite hydrazines, metal nitrate hydrazines, metal perchlorate hydrazines, and mixtures thereof. The complexes within the scope of the present invention rapidly combust or decompose to produce significant quantities of gas.

The metals incorporated within the complexes are transition metals, alkaline earth metals, metalloids, or lanthanide metals that are capable of forming ammine or hydrazine complexes. The presently preferred metal is cobalt. Other metals that also form complexes with the properties desired in the present invention include, for example, magnesium, manganese, nickel, titanium, copper, chromium, zinc, and tin. Examples of other usable metals include rhodium, iridium, ruthenium, palladium, and platinum. These metals are not as preferred as the metals mentioned above, primarily because of cost considerations.

The transition metal cation or alkaline earth metal cation acts as a template at the center of the coordination complex. As mentioned above, the complex includes a neutral ligand containing hydrogen and nitrogen. Currently preferred neutral ligands are  $\text{NH}_3$  and  $\text{N}_2\text{H}_4$ . One or more oxidizing anions may also be coordinated with the metal cation. Examples of metal complexes within the scope of the present invention include  $\text{Cu}(\text{NH}_3)_4(\text{NO}_3)_2$  (tetraamminecopper(II) nitrate),  $\text{Co}(\text{NH}_3)_3(\text{NO}_2)_3$  (trinitrotriamminecobalt(III)),  $\text{Co}(\text{NH}_3)_6(\text{ClO}_4)_3$  (hexaamminecobalt(III) perchlorate),  $\text{Co}(\text{N}_3)_6(\text{NO}_3)_3$  (hexaamminecobalt (III) nitrate),  $\text{Zn}(\text{N}_2\text{H}_4)_3(\text{NO}_3)_2$  (tris-hydrazine zinc nitrate),  $\text{Mg}(\text{N}_2\text{H}_4)_2(\text{ClO}_4)_2$  (bis-hydrazine magnesium perchlorate), and  $\text{Pt}(\text{NO}_2)_2(\text{NH}_2\text{NH}_2)_2$  (bis-hydrazine platinum(II) nitrite).

It is within the scope of the present invention to include metal complexes which contain a common ligand in addition to the neutral ligand. A few typical common ligands include: aquo ( $\text{H}_2\text{O}$ ), hydroxo ( $\text{OH}$ ), carbonato ( $\text{CO}_3$ ), oxalato ( $\text{C}_2\text{O}_4$ ), cyano ( $\text{CN}$ ), isocyanato ( $\text{NC}$ ), chloro ( $\text{Cl}$ ), fluoro ( $\text{F}$ ), and similar ligands. The metal complexes within the scope of the present invention are also intended to include a common counter ion, in addition to the oxidizing anion, to help balance the charge of the complex. A few typical

common counter ions include: hydroxide ( $\text{OH}^-$ ), chloride ( $\text{Cl}^-$ ), fluoride ( $\text{F}^-$ ), cyanide ( $\text{CN}^-$ ), carbonate ( $\text{CO}_3^{2-}$ ), phosphate ( $\text{PO}_4^{3-}$ ), oxalate ( $\text{C}_2\text{O}_4^{2-}$ ), borate ( $\text{BO}_4^{5-}$ ), ammonium ( $\text{NH}_4^+$ ), and the like.

It is observed that metal complexes containing the described neutral ligands and oxidizing anions combust rapidly to produce significant quantities of gases. Combustion can be initiated by the application of heat or by the use of conventional igniter devices.

#### DETAILED DESCRIPTION OF THE INVENTION

As discussed above, the present invention is related to gas generant compositions containing complexes of transition metals or alkaline earth metals. These complexes are comprised of a metal cation template and a neutral ligand containing hydrogen and nitrogen. One or more oxidizing anions are provided to balance the charge of the complex. In some cases the oxidizing anion is part of the coordination complex with the metal cation. Examples of typical oxidizing anions that can be used include nitrates, nitrites, chlorates, perchlorates, peroxides, and superoxides. The complexes can be, combined with a binder or mixture of binders to improve the crush strength and other mechanical properties of the gas generant composition. A co-oxidizer can be provided primarily to permit efficient combustion of the binder.

Metal complexes that include at least one common ligand in addition to the neutral ligand are also included within the scope of, the present invention. As used herein, the term common ligand includes well known ligands used by inorganic chemists to prepare coordination complexes with metal cations. The common ligands are preferably polyatomic ions or molecules, but some monoatomic ions, such as halogen ions, may also be used. Examples of common ligands within the scope of the present invention include aquo ( $\text{H}_2\text{O}$ ), hydroxo ( $\text{OH}$ ), perhydroxo ( $\text{O}_2\text{H}$ ), peroxy ( $\text{O}_2$ ), carbonato ( $\text{CO}_3$ ), oxalato ( $\text{C}_2\text{O}_4$ ), carbonyl ( $\text{CO}$ ), nitrosyl ( $\text{NO}$ ), cyano ( $\text{CN}$ ), isocyanato ( $\text{NC}$ ), isothiocyanato ( $\text{NCS}$ ), thiocyanato ( $\text{SCN}$ ), chloro ( $\text{Cl}$ ), fluoro ( $\text{F}$ ), amido ( $\text{N}(\text{H})_2$ ), imido ( $\text{NH}$ ), sulfato ( $\text{SO}_4$ ), phosphato ( $\text{PO}_4$ ), ethylenediaminetetraacetic acid (EDTA), and similar ligands. See, F. Albert Cotton and Geoffrey Wilkinson, *Advanced Inorganic Chemistry*, 2nd ed., John Wiley & Sons, pp. 139-142, 1966 and James E. Huheey, *Inorganic Chemistry*, 3rd ed., Harper & Row, pp. A-97-A-107, 1983, which are incorporated herein by reference. Persons skilled in the art will appreciate that suitable metal complexes within the scope of the present invention can be prepared containing a neutral ligand and another ligand not listed above.

In some cases, the complex can include a common counter ion, in addition to the oxidizing anion, to help balance the charge of the complex. As used herein, the term common counter ion includes well known anions and cations used by inorganic chemists as counter ions. Examples of common counter ions within the scope of the present invention include hydroxide ( $\text{OH}^-$ ), chloride ( $\text{Cl}^-$ ), fluoride ( $\text{F}^-$ ), cyanide ( $\text{CN}^-$ ), thiocyanate ( $\text{SCN}^-$ ), carbonate ( $\text{CO}_3^{2-}$ ), sulfate ( $\text{SO}_4^{2-}$ ), phosphate ( $\text{PO}_4^{3-}$ ), oxalate ( $\text{C}_2\text{O}_4^{2-}$ ), borate ( $\text{BO}_4^{5-}$ ), ammonium ( $\text{NH}_4^+$ ), and the like. See, Whitten, K. W., and Gailey, K. D., *General Chemistry*, Saunders College Publishing, p. 167, 1981 and James-E. Huheey, *Inorganic Chemistry*, 3rd ed., Harper & Row, pp. A-97- A-103, 1983, which are incorporated herein by reference.

The gas generant ingredients are formulated such that when the composition combusts, nitrogen gas and water

vapor are produced. In some cases, small amounts of carbon dioxide or carbon monoxide are produced if a binder, co-oxidizer, common ligand or oxidizing anion contain carbon. The total carbon in the gas generant composition is carefully controlled to prevent excessive generation of CO gas. The combustion of the gas generant takes place at a rate sufficient to qualify such materials for use as gas-generating compositions in automobile air bags and other similar types of devices. Importantly, the production of other undesirable gases or particulates is substantially reduced or eliminated.

Complexes that fall within the scope of the present invention include metal nitrate ammines, metal nitrite ammines, metal perchlorate ammines, metal nitrite hydrazines, metal nitrate hydrazines, metal perchlorate hydrazines, and mixtures thereof. Metal ammine complexes are defined as coordination complexes including ammonia as the coordinating ligand. The ammine complexes can also have one or more oxidizing anions, such as nitrite ( $\text{NO}_2^-$ ), nitrate ( $\text{NO}_3^-$ ), chlorate ( $\text{ClO}_3^-$ ), perchlorate ( $\text{ClO}_4^-$ ), peroxide ( $\text{O}_2^{2-}$ ), and superoxide ( $\text{O}_2^-$ ), or mixtures thereof, in the complex. The present invention also relates to similar metal hydrazine complexes containing corresponding oxidizing anions.

It is suggested that during combustion of a complex containing nitrite and ammonia groups, the nitrite and ammonia groups undergo a diazotization reaction. This reaction is similar, for example, to the reaction of sodium nitrite and ammonium sulfate, which is set forth as follows:



Compositions such as sodium nitrite and ammonium sulfate in combination have little utility as gas-generating substances. These materials are observed to undergo metathesis reactions, which result in unstable ammonium nitrite. In addition, most simple nitrite salts have limited stability.

In contrast, the metal complexes used in the present invention are stable materials that, in certain instances, are capable of undergoing the type of reaction set forth above. The complexes of the present invention also produce reaction products that include desirable quantities of nontoxic gases, such as water vapor and nitrogen. In addition, a stable metal, or metal oxide slag is formed. Thus, the compositions of the present invention avoid several of the limitations of existing sodium azide gas-generating compositions.

Any transition metal, alkaline earth metal, metalloid, or lanthanide metal capable of forming the complexes described herein is a potential candidate for use in these gas-generating compositions. However, considerations such as cost, reactivity, thermal stability, and toxicity may limit the most preferred group of metals.

The presently preferred metal is cobalt. Cobalt forms stable complexes that are relatively inexpensive. In addition, the reaction products of cobalt complex combustion are relatively nontoxic. Other preferred metals include magnesium, manganese, copper, zinc, and tin. Examples of less preferred but usable metals include nickel, titanium, chromium, rhodium, iridium, ruthenium, and platinum.

A few representative examples of ammine complexes within the scope of the present invention, and the associated gas-generating decomposition reactions are as follows:



A few representative examples of hydrazine complexes within the scope of the present invention, and related gas-generating reactions are as follows:



While the complexes of the present invention are relatively stable, it is also simple to initiate the combustion reaction. For example, if the complexes are contacted with a hot wire, rapid gas producing combustion reactions are observed. Similarly, it is possible to initiate the reaction by means of conventional igniter devices. One type of igniter device includes a quantity of  $\text{B}/\text{KNO}_3$  granules or pellets that is ignited, and which in turn is capable of igniting the compositions of the present invention. Another igniter device includes a quantity of  $\text{Mg}/\text{Sr}(\text{NO}_3)_2/\text{nylon}$  granules.

It is also important to note that many of the complexes defined above undergo "stoichiometric" decomposition. That is, the complexes decompose without reacting with any other material to produce large quantities of nitrogen and water, and a metal or metal oxide. However, for certain complexes it may be desirable to add a fuel or oxidizer to the complex in order to assure complete and efficient reaction. Such fuels include, for example, boron, magnesium, aluminum, hydrides of boron or aluminum, carbon, silicon, titanium, zirconium, and other similar conventional fuel materials, such as conventional organic binders. Oxidizing species include-nitrates, nitrites, chlorates, perchlorates, peroxides, and other similar oxidizing materials. Thus, while stoichiometric decomposition is attractive because of the

simplicity of the composition and reaction, it is also possible to use complexes for which stoichiometric decomposition is not possible.

As mentioned above, nitrate and perchlorate complexes also fall within the scope of the invention. A few representative examples of such nitrate complexes include:  $\text{Co}(\text{NH}_3)_6(\text{NO}_3)_3$ ,  $\text{Cu}(\text{NH}_3)_4(\text{NO}_3)_2$ ,  $[\text{Co}(\text{NH}_3)_5(\text{NO}_2)](\text{NO}_3)_2$ ,  $[\text{Co}(\text{NH}_3)_5(\text{NO}_2)](\text{NO}_3)_2$ ,  $[\text{Co}(\text{NH}_3)_5(\text{H}_2\text{O})](\text{NO}_3)_2$ . A few representative examples of perchlorate complexes within the scope of the invention include:  $[\text{Co}(\text{NH}_3)_6](\text{ClO}_4)_3$ ,  $[\text{Co}(\text{NH}_3)_5(\text{NO}_2)\text{ClO}_4]$ ,  $(\text{Mg}(\text{N}_2\text{H}_4)_2)(\text{ClO}_4)_2$ .

Preparation of metal nitrite or nitrate ammine complexes of the present invention is described in the literature. Specifically, reference is made to Hagel et al., "The Triamines of Cobalt (III). I. Geometrical Isomers of Trinitrotetraminecobalt (III)," 9 *Inorganic Chemistry* 1496 (June 1970); G. Pass and H. Sutcliffe, *Practical Inorganic Chemistry*, 2nd Ed., Chapman & Hull, N.Y., 1974; Shibata et al., "Synthesis of Nitroammine- and Cyanoamminecobalt (III) Complexes With Potassium Tricarbonatocobaltate(III) as the Starting Material," 3 *Inorganic Chemistry* 1573 (November 1964); Wieghardt et al., " $\mu$ -Carboxylatodi- $\mu$ -hydroxo-bis[triamminecobalt (III)] Complexes," 23 *Inorganic Synthesis* 23 (1985); Laing, "mer- and fac-[ $\text{Co}(\text{NH}_3)_3\text{NO}_2)_3$ ] Do They Exist?" 62 *J. Chem Educ.*, 707 (1985); Siebert, "Isomere des Trinitrotetraminecobalt(III)," 441 *Z. Anorg. Allg. Chem.* 47 (1978); all of which are incorporated herein by this reference. Transition metal perchlorate ammine complexes are synthesized by similar methods. As mentioned above, the ammine complexes of the present invention are generally stable and safe for use in preparing gas-generating formulations.

Preparation of metal perchlorate, nitrate, and nitrite hydrazine complexes is also described in the literature. Specific reference is made to Patil et al., "Synthesis and Characterisation of Metal Hydrazine Nitrate, Azide, and Perchlorate Complexes," 12 *Synthesis and Reactivity Inorganic and Metal Organic Chemistry*, 383 (1982); Klyuchnikov et al., "Preparation of Some Hydrazine Compounds of Palladium," 13 *Russian Journal of Inorganic Chemistry*, 416 (1968); Klyuchnikov et al., "Conversion of Mononuclear Hydrazine Complexes of Platinum and Palladium Into Binuclear Complexes," 36 *Ukr. Khim. Zh.*, 687 (1970).

The described complexes can be processed into usable granules or pellets for use in gas-generating devices. Such devices include automobile air bag supplemental restraint systems. Such gas-generating compositions will comprise a quantity of the described complexes and preferably, a binder and a co-oxidizer. The compositions produce a mixture of gases, principally nitrogen and water vapor, upon decomposition or burning. The gas-generating device will also include means for initiating the burning of the composition, such as a hot wire or igniter. In the case of an automobile air bag system, the system will include the compositions described above; a collapsed, inflatable air bag; and means for igniting the gas-generating composition within the air bag system. Automobile air bag systems are well known in the art.

Typical binders used in the gas-generating compositions of the present invention include binders conventionally used in propellant, pyrotechnic and explosive compositions including, but not limited to, lactose, boric acid, silicates, including magnesium silicate, polypropylene carbonate, polyethylene glycol, naturally occurring gums, such as guar gum, acacia gum, modified celluloses and starches (a detailed discussion of such gums is provided by C. L. Mantell, *The Water-Soluble Gums*, Reinhold Publishing

Corp., 1947, which is incorporated herein by reference), polyacrylic acids, nitro-cellulose, polyacrylamide, polyamides, including nylon, and other conventional polymeric binders. Such binders improve, mechanical properties or provide enhanced crush strength. Although water immiscible binders can be used in the present invention, it is currently preferred to use water soluble binders. The binder concentration is preferably in the range from 0.5 to 12% by weight, and more preferably from 2% to 8% by weight of the gas generant composition.

Applicants have found that the addition of carbon, such as carbon black or activated charcoal, to gas generant compositions improves binder action significantly, perhaps by reinforcing the binder and, thus, forming a micro-composite.

Improvements in crush strength of 50% to 150% have been observed with the addition of carbon black to compositions within the scope of the present invention. Ballistic reproducibility is enhanced as crush strength increases. The carbon concentration is preferably in the range of 0.1% to 6% by weight, and more preferably from 0.3 to 3% by weight of the gas generant composition.

The co-oxidizer can be a conventional oxidizer, such as alkali, alkaline earth, lanthanide, or ammonium perchlorates, chlorates, peroxides, nitrites, and nitrates, including for example,  $\text{Sr}(\text{NO}_3)_2$ ,  $\text{NH}_4\text{ClO}_4$ ,  $\text{KNO}_3$ , and  $(\text{NH}_4)_2\text{Ce}(\text{NO}_3)_6$ .

The co-oxidizer can also be a metal-containing oxidizing agent, such as metal oxides, metal hydroxides, metal peroxides, metal oxide hydrates, metal oxide hydroxides, metal hydrous oxides, and mixtures thereof, including those described in U.S. Pat. No. 5,439,537 issued Aug. 8, 1995, titled "Thermite Compositions for Use as Gas Generants," which is incorporated herein by reference. Examples of metal oxides include, among others, the oxides of copper, cobalt, manganese, tungsten, bismuth, molybdenum, and iron, such as  $\text{CuO}$ ,  $\text{CO}_2\text{O}_3$ ,  $\text{CO}_3\text{O}_4$ ,  $\text{CoFe}_2\text{O}_4$ ,  $\text{Fe}_2\text{O}_3$ ,  $\text{MoO}_3$ ,  $\text{Bi}_2\text{MoO}_6$ , and  $\text{Bi}_2\text{O}_3$ . Examples of metal hydroxides include, among others,  $\text{Fe}(\text{OH})_3$ ,  $\text{Co}(\text{OH})_3$ ,  $\text{Co}(\text{OH})_2$ ,  $\text{Ni}(\text{OH})_2$ ,  $\text{Cu}(\text{OH})_2$ , and  $\text{Zn}(\text{OH})_2$ . Examples of metal oxide hydrates and metal hydrous oxides include, among others,  $\text{Fe}_2\text{O}_3 \cdot \text{xH}_2\text{O}$ ,  $\text{SnO}_2 \cdot \text{xH}_2\text{O}$ , and  $\text{MoO}_3 \cdot \text{H}_2\text{O}$ . Examples of metal oxide hydroxides include, among others,  $\text{CoO}(\text{OH})_2$ ,  $\text{FeO}(\text{OH})_2$ ,  $\text{MnO}(\text{OH})_2$  and  $\text{MnO}(\text{OH})_3$ .

The co-oxidizer can also be a basic metal carbonate, such as metal carbonate hydroxides, metal carbonate oxides, metal carbonate hydroxide oxides, and hydrates and mixtures thereof and a basic metal nitrate, such as metal hydroxide nitrates, metal nitrate oxides, and hydrates and mixtures thereof, including those oxidizers described in U.S. Pat. No. 5,429,691, titled "Thermite Compositions for use as Gas Generants," which is incorporated herein by reference.

Table 1, below, lists examples of typical basic metal carbonates capable of functioning as co-oxidizers in the compositions of the present invention:

TABLE 1

| Basic Metal Carbonates                                                                                                                          |
|-------------------------------------------------------------------------------------------------------------------------------------------------|
| $\text{Cu}(\text{CO}_3)_{1-x}\text{Cu}(\text{OH})_{2x}$ , e.g., $\text{CuCO}_3\text{Cu}(\text{OH})_2$ (malachite)                               |
| $\text{Co}(\text{CO}_3)_{1-x}(\text{OH})_{2x}$ , e.g., $2\text{Co}(\text{CO}_3)_3\text{Co}(\text{OH})_2\text{H}_2\text{O}$                      |
| $\text{Co}_x\text{Fe}_y(\text{CO}_3)_2(\text{OH})_2$ , e.g., $\text{Co}_{0.69}\text{Fe}_{0.34}(\text{CO}_3)_{0.2}(\text{OH})_2$                 |
| $\text{Na}_3[\text{Co}(\text{CO}_3)_3]_3\text{H}_2\text{O}$                                                                                     |
| $\text{Zn}(\text{CO}_3)_{1-x}(\text{OH})_{2x}$ , e.g., $\text{Zn}_2(\text{CO}_3)(\text{OH})_2$                                                  |
| $\text{Bi}_A\text{Mg}_B(\text{CO}_3)_C(\text{OH})_D$ , e.g., $\text{Bi}_2\text{Mg}(\text{CO}_3)_2(\text{OH})_4$                                 |
| $\text{Fe}(\text{CO}_3)_{1-x}(\text{OH})_{2x}$ , e.g., $\text{Fe}(\text{CO}_3)_{0.12}(\text{OH})_{2.76}$                                        |
| $\text{Cu}_{2-x}\text{Zn}_x(\text{CO}_3)_{1-y}(\text{OH})_{2y}$ , e.g., $\text{Cu}_{1.54}\text{Zn}_{0.46}(\text{CO}_3)(\text{OH})_2$            |
| $\text{Co}_y\text{Cu}_{2-y}(\text{CO}_3)_{1-x}(\text{OH})_{2x}$ , e.g., $\text{Co}_{0.49}\text{Cu}_{0.51}(\text{CO}_3)_{0.43}(\text{OH})_{1.1}$ |

TABLE 1-continued

| Basic Metal Carbonates                                                                                       |   |  |
|--------------------------------------------------------------------------------------------------------------|---|--|
| $Ti_A Bi_B (CO_3)_x (OH)_y (O_z (H_2O)_c$ , e.g., $Ti_3 Bi_4 (CO_3)_2 (OH)_2 O_9 (H_2O)_2$<br>$(BiO)_2 CO_3$ | 5 |  |

Table 2, below, lists examples of typical basic metal nitrates capable of functioning as co-oxidizers in the compositions of the present invention:

TABLE 2

| Basic Metal Nitrates                                              |    |  |
|-------------------------------------------------------------------|----|--|
| $Cu_2 (OH)_3 NO_3$ (gerhardtite)                                  | 10 |  |
| $Co_2 (OH)_3 NO_3$                                                |    |  |
| $Cu_x Co_{2-x} (OH)_3 NO_3$ , e.g., $CuCo(OH)_3 NO_3$             |    |  |
| $Zn_2 (OH)_3 NO_3$                                                | 15 |  |
| $Mn(OH)_2 NO_3$                                                   |    |  |
| $Fe(NO_3)_n (OH)_{3-n}$ , e.g., $Fe_4 (OH)_{11} NO_3 \cdot 2H_2O$ |    |  |
| $Mo(NO_3)_2 O_2$                                                  |    |  |
| $BiONO_3 \cdot H_2O$                                              |    |  |
| $Ce(OH)(NO_3)_3 \cdot 3H_2O$                                      |    |  |

In certain instances it will also be desirable to use mixtures of such oxidizing agents in order to enhance ballistic properties or maximize filterability of the slag formed from combustion of the composition.

The present compositions can also include additives conventionally used in gas-generating compositions, propellants, and explosives, such as burn rate modifiers, slag formers, release agents, and additives that effectively remove  $NO_x$ . Typical burn-rate modifiers include  $Fe_2O_3$ ,  $K_2B_{12}H_{12}$ ,  $Bi_2MoO_6$ , and graphite carbon powder or fibers. A number of slag forming agents are known and include, for example, clays, talcs, silicon oxides, alkaline earth oxides, hydroxides, oxalates, of which magnesium carbonate, and magnesium hydroxide are exemplary. A number of additives and/or agents are also known to reduce or eliminate the oxides of nitrogen from the combustion products of a gas generant composition, including alkali metal salts and complexes of tetrazoles, aminotetrazoles, triazoles and related nitrogen heterocycles of which potassium aminotetrazole, sodium carbonate and potassium carbonate are exemplary. The composition can also include materials that facilitate the release of the composition from a mold such as graphite, molybdenum sulfide, calcium stearate, or boron nitride.

Typical ignition aids/burn rate modifiers that can be used herein include metal oxides, nitrates and other compounds, such as, for instance,  $Fe_2O_3$ ,  $K_2B_{12}H_{12} \cdot H_2O$ ,  $BiO(NO_3)_3$ ,  $CO_2O_3$ ,  $CoFe_2O_4$ ,  $CuMoO_4$ ,  $Bi_2MoO_6$ ,  $MnO_2$ ,  $Mg(NO_3)_2 \cdot xH_2O$ ,  $Fe(NO_3)_3 \cdot xH_2O$ ,  $Co(NO_3)_2 \cdot xH_2O$ , and  $NH_4NO_3$ . Coolants include magnesium hydroxide, cupric oxalate, boric acid, aluminum hydroxide, and silicotungstic acid. Coolants such as aluminum hydroxide and silicotungstic acid can also function as slag enhancers.

It will be appreciated that many of the foregoing additives may perform multiple functions in the gas generant formulation, such as a co-oxidizer or as a fuel, depending on the compound. Some compounds may function as a co-oxidizer, burn-rate modifier, coolant, and/or slag former.

Several important properties of typical hexaamminecobalt (III) nitrate gas generant compositions within the scope of the present invention have been compared with those of commercial sodium azide gas generant compositions. These properties illustrate significant differences between conventional sodium azide gas generant composi-

tions and gas generant compositions within the scope of the present invention. These properties are summarized below:

| Property                          | Typical Invention Range    | Typical Sodium Azide        |
|-----------------------------------|----------------------------|-----------------------------|
| Flame Temperature                 | 1850–2050° K.              | 1400–1500° K.               |
| Gas Fraction of Generant          | 0.65–0.85                  | 0.4–0.45                    |
| Total Carbon Content in Generant  | 0–3.5%                     | trace                       |
| Burn Rate of Generant at 1000 psi | 0.10–0.35 ips              | 1.1–1.3 ips                 |
| Surface Area of Generant          | 2.0–3.5 cm <sup>2</sup> /g | 0.8–0.85 cm <sup>2</sup> /g |
| Charge Weights in Generator       | 30–45 g                    | 75–90 g                     |

The term "gas fraction of generant" means the weight fraction of gas generated per weight of gas generant. Typical hexaamminecobalt(III) nitrate gas generant compositions have more preferred flame temperatures in the range from 1850° K to 1900° K, gas fraction of generant in the range from 0.70 to 0.75, total carbon content in the generant in the range from 1.5% to 3.0%, burn rate of generant at 1000 psi in the range from 0.2 ips to 0.35 ips, and surface area of generant in the range from 2.5 cm<sup>2</sup>/g to 3.5 cm<sup>2</sup>/g.

The gas-generating compositions of the present invention are readily adapted for use with conventional hybrid air bag inflator technology. Hybrid inflator technology is based on heating a stored inert gas (argon or helium) to a desired temperature by burning a small amount of propellant. Hybrid inflators do not require cooling filters used with pyrotechnic inflators to cool combustion gases, because hybrid inflators are able to provide a lower temperature gas. The gas discharge temperature can be selectively changed by adjusting the ratio of inert gas weight to propellant weight. The higher the gas weight to propellant weight ratio, the cooler the gas discharge temperature.

A hybrid gas-generating system comprises a pressure tank having a rupturable opening, a pre-determined amount of inert gas disposed within that pressure tank; a gas-generating device for producing hot combustion gases and having means for rupturing the rupturable opening; and means for igniting the gas-generating composition. The tank has a rupturable opening, which can be broken by a piston when, the gas-generating device is ignited. The gas-generating device is configured and positioned relative to the pressure-tank so that hot combustion gases are mixed with and heat the inert gas. Suitable inert gases include, among others, argon, helium and mixtures thereof. The mixed and heated gases exit the pressure tank through the opening and ultimately exit the hybrid inflator and deploy an inflatable bag or balloon, such as an automobile air bag.

Preferred embodiments of the invention yield combustion products with a temperature greater than about 180° K, the heat of which is transferred to the cooler inert gas causing a further improvement in the efficiency of the hybrid gas-generating system.

Hybrid gas-generating devices for supplemental safety restraint application are described in Frantom, Hybrid Airbag Inflator Technology, *Airbag Int/Symposium on Sophisticated Car Occupant Safety Systems*, (Weinbrenner-Saal, Germany, Nov. 2–3, 1992).

## 11

## EXAMPLES

The present invention is further described in the following non-limiting examples. Unless otherwise stated, the compositions are expressed in weight percent.

## Example 1

A quantity (132.4 g) of  $\text{Co}(\text{NH}_3)_3(\text{NO}_2)_3$ , prepared according to the teachings of Hagel et al., "The Triamines of Cobalt (III). I. Geometrical Isomers of Trinitrotriamminecobalt(III)," 9 Inorganic Chemistry, 1496 (June 1970), was slurried in 35 mL of methanol with 7 g of a 38 percent by weight solution of pyrotechnic grade vinyl acetate/vinyl alcohol polymer resin commonly known as VAAR dissolved in methyl acetate. The solvent was allowed to partially evaporate. The paste-like mixture was forced through a 20-mesh sieve, allowed to dry to a stiff consistency, and forced through a sieve yet again. The granules resulting were then dried in vacuo at ambient temperature for 12 hours. One-half-inch diameter pellets of the dried material were prepared by pressing. The pellets were combusted at several different pressures ranging from 600 to 3,300 psig. The burning rate of the generant was found to be 0.237 inch per second at 1,000 psig with a pressure exponent of 0.85 over the pressure range tested.

## Example 2

The procedure of Example 1 was repeated with 100 g of  $\text{Co}(\text{NH}_3)_3(\text{NO}_2)_3$  and 34 g of 12 percent by weight solution of nylon in methanol. Granulation was accomplished via 10- and 16-mesh screens followed by air drying. The burn rate of this composition was found to be 0.290 inch per second at 1,000 psig with a pressure exponent of 0.74.

## Example 3

In a manner similar to that described in Example 1, 400 g of  $\text{Co}(\text{NH}_3)_3(\text{NO}_2)_3$  was slurried with 219 g of a 12 percent by weight solution of nitrocellulose in acetone. The nitrocellulose contained 12.6 percent nitrogen. The solvent was allowed to partially evaporate. The resulting paste was forced through an 8-mesh sieve followed by a 24-mesh sieve. The resultant granules were dried in air overnight and blended with sufficient calcium stearate mold release agent to provide 0.3 percent by weight in the final product. A portion of the resulting material was pressed into 0.5-inch diameter pellets and found to exhibit a burn rate of 0.275 inch per second at 1,000 psig with a pressure exponent of 0.79. The remainder of the material was pressed into pellets 0.125-inch diameter by 0.07-inch thickness on a rotary tablet press. The pellet density was determined to be 1.88 g/cc. The theoretical flame temperature of this composition was 2,358° K and was calculated to provide a gas mass fraction of 0.72.

## Example 4

This example discloses the preparation of a reusable stainless steel test fixture used to simulate driver's side gas generators. The test fixture, or simulator, consisted of an igniter chamber and a combustion chamber. The igniter chamber was situated in the center and had 24, 0.10-inch diameter ports exiting into the combustion chamber. The igniter chamber was fitted with an igniter squib. The igniter chamber wall was lined with 0.001-inch thick aluminum foil before -24/+60-mesh igniter granules were added. The outer combustion chamber wall consisted of a ring with nine exit ports. The diameter of the ports was varied by changing

## 12

rings. Starting from the inner diameter of the outer combustion chamber ring, the combustion chamber was fitted with a 0.004-inch aluminum shim, one wind of 30-mesh stainless steel screen, four winds of a 14-mesh stainless steel screen, 5 a deflector ring, and the gas generant. The generant was held intact in the combustion chamber using a "donut" of 18-mesh stainless steel screen. An additional deflector ring was placed around the outside diameter of the outer combustion chamber wall. The combustion chamber was fitted with a pressure port. The simulator was attached to either a 60-liter tank or an automotive air bag. The tank was fitted with pressure, temperature, vent, and drain ports. The automotive air bags have a maximum capacity of 55 liters and are constructed with two 0.5-inch diameter vent ports. Simulator tests involving an air bag were configured such that bag pressures were measured. The external skin surface temperature of the bag was monitored during the inflation event by infrared radiometry, thermal imaging, and thermocouple.

## Example 5

Thirty-seven and one-half grams of the 0.125-inch diameter pellets prepared as described in Example 3 were combusted in an inflator test device vented into a 60-L collection tank as described in Example 4, with the additional incorporation of a second screened chamber containing two winds of 30-mesh screen and two winds of 18-mesh screen. The combustion produced a combustion chamber pressure of 2,000 psia and a pressure of 39 psia in the 60-L collection tank. The temperature of the gases in the collection tank reached a maximum of 670° K at 20 milliseconds. Analysis of the gases collected in the 60-L tank showed a concentration of nitrogen oxides ( $\text{NO}_x$ ) of 500 ppm and a concentration of carbon monoxide of 1,825 ppm. Total expelled particulate as determined by rinsing the tank with methanol and evaporation of the rinse was found to be 1,000 mg.

## Example 6

The test of Example 4 was repeated, except that the 60-L tank was replaced with a 55-L vented bag as typically employed in driver side automotive inflator restraint devices. A combustion chamber pressure of 1,900 psia was obtained with a full inflation of the bag occurring. An internal bag pressure of 2 psig at peak was observed at approximately 60 milliseconds after ignition. The bag surface temperature was observed to remain below 83° C., which is an improvement over conventional azide-based inflators, while the bag inflation performance is quite typical of conventional systems.

## Example 7

The nitrate salt of copper tetraammine was prepared by dissolving 116.3 g of copper(II) nitrate hemipentahydrate in 230 mL of concentrated ammonium hydroxide and 50 mL of water. Once the resulting warm mixture had cooled to 40° C., one liter of ethanol was added with stirring to precipitate the tetraammine nitrate product. The dark purple-blue solid was collected by filtration, washed with ethanol, and air dried. The product was confirmed to be  $\text{Cu}(\text{NH}_3)_4(\text{NO}_3)_2$  by elemental analysis. The burning rate of this material as determined from pressed 0.5-inch diameter pellets was 0.18 inch per second at 1,000 psig.

## Example 8

The tetraammine copper nitrate prepared in Example 7 was formulated with various supplemental oxidizers and

## 13

tested for burning rate. In all cases, 10 g of material were slurred with approximately 10 mL of methanol, dried, and pressed into 0.5-inch diameter pellets. Burning rates were measured at 1,000 psig, and the results are shown in the following table.

| Copper Tetraammine Nitrate | Oxidizer                               | Burn Rate (ips) |
|----------------------------|----------------------------------------|-----------------|
| 88%                        | CuO (6%)                               | 0.13            |
| 92%                        | Sr(NO <sub>3</sub> ) <sub>2</sub> (6%) | 0.14            |
| 90%                        | NH <sub>4</sub> NO <sub>3</sub> (10%)  | 0.25            |
| 78%                        | Bi <sub>2</sub> O <sub>3</sub> (22%)   | 0.10            |
| 85%                        | SrO <sub>2</sub> (15%)                 | 0.18            |

## Example 9

A quantity of hexaamminecobalt (III) nitrate was prepared by replacing ammonium chloride with ammonium nitrate in the procedure for preparing of hexaamminecobalt(III) chloride as taught by G. Pass and H. Sutcliffe, *Practical Inorganic Chemistry*, 2nd Ed., Chapman & Hull, N. Y., 1974. The material prepared was determined to be [Co(NH<sub>3</sub>)<sub>6</sub>](NO<sub>3</sub>)<sub>3</sub> by elemental analysis. A sample of the material was pressed into 0.5-inch diameter pellets and a burning rate of 0.26 inch per second measured at 2,000 psig.

## Example 10

The material prepared in Example 9 was used to prepare three lots of gas generant containing hexaamminecobalt(III) nitrate as the fuel and ceric ammonium nitrate as the co-oxidizer. The lots differ in mode of processing and the presence or absence of additives. Burn rates were determined from 0.5-inch diameter burn rate pellets. The results are summarized below:

| Formulation                                                             | Processing           | Burn Rate   |
|-------------------------------------------------------------------------|----------------------|-------------|
| 12% (NH <sub>4</sub> ) <sub>2</sub> Ce(NO <sub>3</sub> ) <sub>6</sub>   | Dry Mix              | 0.19 ips    |
| 88% [Co(NH <sub>3</sub> ) <sub>6</sub> ](NO <sub>3</sub> ) <sub>3</sub> |                      | at 1690 psi |
| 12% (NH <sub>4</sub> ) <sub>2</sub> Ce(NO <sub>3</sub> ) <sub>6</sub>   | Mixed with           | 0.20 ips    |
| 88% [Co(NH <sub>3</sub> ) <sub>6</sub> ](NO <sub>3</sub> ) <sub>3</sub> | 35% MeOH             | at 1690 psi |
| 18% (NH <sub>4</sub> ) <sub>2</sub> Ce(NO <sub>3</sub> ) <sub>6</sub>   | Mixed with           | 0.20 ips    |
| 81% [Co(NH <sub>3</sub> ) <sub>6</sub> ](NO <sub>3</sub> ) <sub>3</sub> | 10% H <sub>2</sub> O | at 1690 psi |
| 1% Carbon Black                                                         |                      |             |

## Example 11

The material prepared in Example 9 was used to prepare several 10-g mixes of generant compositions utilizing various supplemental oxidizers. In all cases, the appropriate amount of hexaamminecobalt(III) nitrate and co-oxidizer(s) were blended into approximately 10 mL of methanol, allowed to dry, and pressed into 0.5-inch diameter pellets. The pellets were tested for burning rate at 1,000 psig, and the results are shown in the following table.

| Hexaamminecobalt (III) Nitrate | Co-oxidizer | Burning Rate @ 1,000 psig |
|--------------------------------|-------------|---------------------------|
| 60%                            | CuO (40%)   | 0.15                      |
| 70%                            | CuO (30%)   | 0.16                      |

## 14

-continued

|   | Hexaamminecobalt (III) Nitrate | Co-oxidizer                             | Burning Rate @ 1,000 psig |
|---|--------------------------------|-----------------------------------------|---------------------------|
| 5 | 83%                            | CuO (10%)                               | 0.13                      |
|   |                                | Sr(NO <sub>3</sub> ) <sub>2</sub> (7%)  |                           |
|   | 88%                            | Sr(NO <sub>3</sub> ) <sub>2</sub> (12%) | 0.14                      |
|   | 70%                            | Bi <sub>2</sub> O <sub>3</sub> (30%)    | 0.10                      |
|   | 83%                            | NH <sub>4</sub> NO <sub>3</sub> (17%)   | 0.15                      |

## Example 12

Binary compositions of hexaamminecobalt(III) nitrate ("HACN") and various supplemental oxidizers were blended in 20 gram batches. The compositions were dried for 72 hours at 200° F. and pressed into 0.5-inch diameter pellets. Burn rates were determined by burning the ½-inch pellets at different pressures ranging from 1000 to 4000 psi. The results are shown in the following table.

| Composition                                                               | R <sub>b</sub> (ips) at X psi |      |      |      | Temp. ° K. |
|---------------------------------------------------------------------------|-------------------------------|------|------|------|------------|
|                                                                           | 1000                          | 2000 | 3000 | 4000 |            |
| Weight Ratio                                                              |                               |      |      |      |            |
| HACN                                                                      | 0.19                          | 0.28 | 0.43 | 0.45 | 1856       |
| 100/0                                                                     |                               |      |      |      |            |
| HACN/CuO                                                                  | 0.26                          | 0.35 | 0.39 | 0.44 | 1861       |
| 90/10                                                                     |                               |      |      |      |            |
| HACN/[Ce(NH <sub>4</sub> ) <sub>2</sub> (NO <sub>3</sub> ) <sub>6</sub> ] | 0.16                          | 0.22 | 0.30 | 0.38 | —          |
| 88/12                                                                     |                               |      |      |      |            |
| HACN/Co <sub>2</sub> O <sub>3</sub>                                       | 0.10                          | 0.21 | 0.26 | 0.34 | 1743       |
| 90/10                                                                     |                               |      |      |      |            |
| HACN/[Co(NO <sub>3</sub> ) <sub>2</sub> .6H <sub>2</sub> O]               | 0.13                          | 0.22 | 0.35 | 0.41 | 1865       |
| 90/10                                                                     |                               |      |      |      |            |
| HACN/V <sub>2</sub> O <sub>5</sub>                                        | 0.12                          | 0.16 | 0.21 | 0.30 | 1802       |
| 85/15                                                                     |                               |      |      |      |            |
| HACN/Fe <sub>2</sub> O <sub>3</sub>                                       | 0.12                          | 0.12 | 0.17 | 0.23 | 1626       |
| 75/25                                                                     |                               |      |      |      |            |
| HACN/Co <sub>3</sub> O <sub>4</sub>                                       | 0.13                          | 0.20 | 0.25 | 0.30 | 1768       |
| 81.5/18.5                                                                 |                               |      |      |      |            |
| HACN/MnO <sub>2</sub>                                                     | 0.11                          | 0.17 | 0.22 | 0.30 | —          |
| 80/20                                                                     |                               |      |      |      |            |
| HACN/[Fe(NO <sub>3</sub> ) <sub>2</sub> .9H <sub>2</sub> O]               | 0.14                          | 0.22 | 0.31 | 0.48 | —          |
| 90/10                                                                     |                               |      |      |      |            |
| HACN/[Al(NO <sub>3</sub> ) <sub>2</sub> .6H <sub>2</sub> O]               | 0.10                          | 0.18 | 0.26 | 0.32 | 1845       |
| 90/10                                                                     |                               |      |      |      |            |
| HACN/[Mg(NO <sub>3</sub> ) <sub>2</sub> .2H <sub>2</sub> O]               | 0.16                          | 0.24 | 0.32 | 0.39 | 2087       |
| 90/10                                                                     |                               |      |      |      |            |

## Example 13

50 A processing method was devised for preparing small parallelepipeds ("pps.") of gas generant on a laboratory scale. The equipment necessary for forming and cutting the pps. included a cutting table, a roller and a cutting device. The cutting table consisted of a 9 inch×18 inch sheet of 0.35 metal with 0.5-inch wide paper spacers taped along the lengthwise edges. The spacers had a cumulative height of 0.043 inch. The roller consisted of a 1 foot long, 2-inch diameter cylinder of teflon. The cutting device consisted of a shaft, cutter blades and spacers. The shaft was a 0.25-inch bolt upon which a series of seventeen 0.75-inch diameter, 0.005-inch thick stainless steel washers were placed as cutter blades. Between each cutter blade, four 0.66-inch diameter, 0.020-inch thick brass spacer washers were placed and the series of washers were secured by means of a nut. The repeat distance between the circular cutter blades was 0.085-inch.

55 60 65 60 A gas generant composition containing a water-soluble a binder was dry-blended and then 50–70 g batches were

## 15

mixed on a Spex mixer/mill for five minutes with sufficient water so that the material when mixed had a dough-like consistency.

A sheet of velostat plastic was taped to the cutting table and the dough ball of generant mixed with water was flattened by hand onto the plastic. A sheet of polyethylene plastic was placed over the generant mix. The roller was positioned parallel to the spacers on the cutting table and the dough was flattened to a width of about 5 inches. The roller was then rotated 90 degrees, placed on top of the spacers, and the dough was flattened to the maximum amount that the cutter table spacers would allow. The polyethylene plastic was peeled carefully off the generant and the cutting device was used to cut the dough both lengthwise and width-0.25 wise.

The velostat plastic sheet upon which the generant had been rolled and cut was unfastened from the cutting table and placed lengthwise over a 4-inch diameter cylinder in a 135° F. convection oven. After approximately 10 minutes, the sheet was taken out of the oven and placed over a 0.5-inch diameter rod so that the two ends of the plastic sheet formed an acute angle relative to the rod. The plastic was moved back and forth over the rod so as to open up the cuts between the parallelepipeds ("pps."). The sheet was placed widthwise over the four-inch diameter cylinder in the 135° F. convection oven and allowed to dry for another 5 minutes. The cuts were opened between the pps. over the 0.5-inch diameter rod as before. By this time, it was quite easy to detach the pps. from the plastic. The pps. were separated from each other further by rubbing them gently in a pint cup or on the screens of a 12-mesh sieve. This method breaks the pps. into singlets with some remaining doublets. The doublets were split into singlets by use of a razor blade. The pps. were then placed in a convection oven at 165–225° F. to dry them completely. The crush strengths (on edge) of the pps. thus formed were typically as great or greater than those of 0.125-inch diameter pellets with a 0.25-inch convex radius of curvature and a 0.070-inch maximum height that were formed on a rotary-press. This is noteworthy since the latter are three times as massive.

## Example 14

A gas-generating composition was prepared utilizing hexaamminecobalt(III) nitrate,  $[\text{NH}_3]_6\text{Co}(\text{NO}_3)_3$ , powder (78.07%, 39.04 g), ammonium nitrate granules (19.93's, 9.96 g), and ground polyacrylamide, MW 15 million (2.00%, 1.00 g). The ingredients were dry-blended in a Spex mixer/mill for one minute. Deionized water (129 of the dry weight of the formulation, 6 g) was added to the mixture, which was blended for an additional five minutes on the Spex mixer/mill. This resulted in material with a dough-like consistency, which was processed into parallelepipeds (pps.) as in Example 13. Three additional batches of generant were mixed and processed similarly. The pps. from the four batches were blended. The dimensions of the pps. were 0.052 inch×0.072 inch×0.084 inch. Standard-deviations on each of the dimensions were on the order of 0.010 inch. The average weight of the pps. was 6.62 mg. The bulk density, density as determined by dimensional measurements, and density as determined by solvent displacement were determined to be 0.86 g/cc, 1.28 g/cc, and 1.59 g/cc, respectively. Crush strengths of 1.7 kg (on the narrowest edge) were measured with a standard deviation of 0.7 kg. Some of the pps. were pressed into 0.5-inch diameter pellets weighing approximately three grams. From these pellets the burn rate was determined to be 0.13 ips at 1000 psi with a pressure exponent of 0.78.

## 16

## Example 15

A simulator was constructed according to Example 4. Two grams of a stoichiometric blend of  $\text{Mg/Sr}(\text{NO}_3)_2$ /nylon igniter granules were placed into the igniter chamber. The diameter of the ports exiting the outer combustion chamber wall were 0.1875-inch. Thirty grams of generant described in Example 14 in the form of parallelepipeds were secured in the combustion chamber. The simulator was attached to the 60-L tank described in Example 4. After ignition, the combustion chamber reached a maximum pressure of 2300 psia in 17 milliseconds, the 60-L tank reached a maximum pressure of 34 psia and the maximum tank temperature was 640° K. The  $\text{NO}_x$ , CO and  $\text{NH}_3$  levels were 20, 380, and 170 ppm, respectively, and 1600 mg of particulate were collected from the tank.

## Example 16

A simulator was constructed with the exact same igniter and generant type and charge weight as in Example 15. In addition, the outer combustion chamber exit port diameters were identical. The simulator was attached to an automotive safety bag of the type described in Example 4. After ignition, the combustion chamber reached a maximum pressure of 2000 psia in 15 milliseconds. The maximum pressure of the inflated air bag was 0.9 psia. This pressure was reached 18 milliseconds after ignition. The maximum bag surface temperature was 67° C.

## Example 17

A gas-generating composition was prepared utilizing hexaamminecobalt(III) nitrate powder (76.29%, 76.29 g), ammonium nitrate granules (15.71%, 15.71 g, Dynamit Nobel, granule size: <350 micron), cupric oxide powder formed pyrometallurgically (5.00%, 5.00 g) and guar gum (3.00%, 3.00 g). The 36 ingredients were dry-blended in a Spex mixer/mill for one minute. Deionized water (18% of the dry weight of the formulation, 9 g) was added to 50 g of the mixture which was blended for an additional five minutes on the Spex mixer/mill. This resulted in material with a dough-like consistency which was processed into parallelepipeds (pps.) as in Example 13. The same process was repeated for the other 50 g of dry-blended generant and the two batches of pps. were blended together. The average dimensions of the blended pps. were 0.070 inch×0.081 inch×0.088 inch. Standard deviations on each of the dimensions were on the order of 0.010 inch. The average weight of the pps. was 9.60 mg. The bulk density, density as determined by dimensional measurements, and density as determined by solvent displacement were determined to be 0.96 g/cc, 1.17 g/cc, and 1.73 g/cc, respectively. Crush strengths of 5.0 kg (on the narrowest edge) were measured with a standard deviation of 2.5 kg. Some of the pps. were pressed into 0.5-inch diameter pellets weighing approximately three grams. From these pellets the burn rate was determined to be 0.20 ips at 1000 psi with a pressure exponent of 0.67.

## Example 18

A simulator was constructed according to Example 4. One gram of a stoichiometric blend of  $\text{Mg/Sr}(\text{NO}_3)_2$ /nylon and two grams of slightly over-oxidized  $\text{B/KNO}_3$  igniter granules were blended and placed into the igniter chamber. The diameter of the ports exiting the outer combustion chamber wall were 0.166 inch. Thirty grams of generant described in Example 17 in the form of parallelepipeds (pps.) were

17

secured in the combustion chamber. The simulator was attached to the 60-L tank described in Example 4. After ignition, the combustion chamber reached a maximum pressure of 2540 psia in 8 milliseconds, the 60-L tank reached a maximum pressure of 36 psia and the maximum tank temperature was 600° K. The NO<sub>x</sub>, CO, and NH<sub>3</sub> levels were 50, 480, and 800 ppm, respectively, and 240 mg of particulate were collected from the tank.

Example 19

A simulator was constructed with the exact same igniter and generant type and charge weight as in Example 18. In addition the outer combustion chamber exit port diameters were identical. The simulator was attached to an automotive safety bag of the type described in Example 4. After ignition, the combustion chamber reached a maximum pressure of 2700 psia in 9 milliseconds. The maximum pressure of the inflated air bag was 2.3 psig. This pressure was reached 30 milliseconds after ignition. The maximum bag surface temperature was 73° C.

Example 20

A gas-generating composition was prepared utilizing hexaamminecobalt(III) nitrate powder (69.5%, 347.5 g) copper (II) trihydroxy nitrate, 34cu (OH)<sub>3</sub>NO<sub>3</sub>, powder (21.58, 107.5 g), 10 micron RDX (5.00%, 25 g), 26 micron potassium nitrate (1.00%, 5 g) and guar gum (3.00%, 3.00 g). The ingredients were dry-blended with the assistance of a 60-mesh sieve. Deionized water (23% of the dry weight of the formulation, 15 g) was added to 65 g of the mixture, which was blended for an additional five minutes on the Spex mixer/mill. This resulted in material with a dough-like consistency that was processed into parallelepipeds (pps.) as in Example 13. The same process was repeated for two additional 65 g batches of dry-blended generant and the three batches of pps. were blended together. The average dimensions of the pps. were 0.057 inch×0.078 inch×0.084 inch. Standard deviations on each of the dimensions were on the order of 0.010 inch. The average weight of the pps. was 7.22 mg. The bulk density, density as determined by dimensional measurements, and density as determined by solvent displacement were determined to be 0.96 g/cc, 1.23 g/cc, and 1.74 g/cc, respectively. Crush strengths of 3.6 kg (on the narrowest edge) were measured with a standard deviation of 0.9 kg. Some of the pps. were pressed into 0.5-inch diameter pellets weighing approximately three grams. From these pellets the burn rate was determined to be 0.27 ips at 1000 psi with a pressure exponent of 0.51.

Example 21

A simulator was constructed according to Example 4. A stoichiometric blend of 1.5 grams of Mg/Sr(NO<sub>3</sub>)<sub>2</sub>/nylon and 1.5 grams of slightly over-oxidized B/KNO<sub>3</sub> igniter granules were blended and placed into the igniter chamber. The diameter of the ports exiting the outer combustion chamber wall were 0.177 inch. Thirty grams of generant described in Example 20 in the form of parallelepipeds (pps.) were secured in the combustion chamber. The simulator was attached to the 60-L tank described in Example 4. After ignition, the combustion chamber reached a maximum pressure of 3050 psia in 14 milliseconds. The NO<sub>x</sub>, CO, and NH<sub>3</sub> levels were 25, 800, and 90 ppm, respectively, and 890 mg of particulate were collected from the tank.

18

Example 22

A gas-generating composition was prepared utilizing hexaamminecobalt(III) nitrate powder (78.00%, 457.9 g), copper(II) trihydroxy nitrate powder (19.00%, 111.5 g), and guar gum (3.00%, 17.61 g). The ingredients were dry-blended and then, mixed with water (32.5% of the dry weight of the formulation, 191 g) in a Baker-Perkins pint mixer for 30 minutes. To a portion of the resulting wet cake (220 g), 9.2 additional grams of copper(II) trihydroxy nitrate and 0.30 additional grams of guar gum were added, as well as 0.80 g of carbon black (Monarch 1100). This new formulation was blended for 30 minutes on a Baker-Perkins mixer. The wet cake was placed in a ram extruder with a barrel diameter of 2 inches and a die orifice diameter of 3/32 inch (0.09038 inch). The extruded material was cut into lengths of about one foot, allowed to dry under ambient conditions overnight, placed into an enclosed container-holding water in order to moisten and thus soften the material, chopped into lengths of about 0.1 inch and dried at 165° F. The dimensions of the resulting extruded cylinders were an average length of 0.113 inch and an average diameter of 0.091 inch. The bulk density, density as determined by dimensional measurements, and density as determined by solvent displacement were 0.86 g/cc, 1.30 g/cc, and 1.61 g/cc; respectively. Crush strengths of 2.1 and 4.1 kg were measured on the circumference and axis, respectively. Some of the extruded cylinders were pressed into 0.5-inch diameter pellets weighing approximately three grams. From these pellets the burn rate was determined to be 0.22 ips at 1000 psi with a pressure exponent of 0.29.

Example 23

Three simulators were constructed according to Example 4. A stoichiometric blend of 1.5 grams of Mg/Sr(NO<sub>3</sub>)<sub>2</sub>/nylon and 1.5 grams of slightly over-oxidized B/KNO<sub>3</sub> igniter granules were blended and placed into the igniter chambers. The diameter of the ports exiting the outer combustion chamber wall were 0.177 inch, 0.166 inch, and 0.152 inch, respectively. Thirty grams of generant described in Example 22 in the form of extruded cylinders were secured in each of the combustion chambers. The simulators were, in succession, attached to the 60-L tank described in Example 4. After ignition, the combustion chambers reached a maximum pressure of 1585, 1665, and 1900 psia, respectively. Maximum tank pressures were 32, 34, and 35 psia, respectively. The NO<sub>x</sub> levels were 85, 180, and 185 ppm whereas the CO levels were 1540, 600, and 600 ppm, respectively. NH<sub>3</sub> levels were below 2 ppm. Particulate levels were 420, 350, and 360 mg, respectively.

Example 24

The addition of small amounts of carbon to gas generant formulations have been found to improve the crush strength of parallelepipeds and extruded pellets formed as in Example 13 or Example 22. The following table summarizes the crush strength enhancement with the addition of carbon to a typical gas generant composition within the scope of the present invention. All percentages are expressed as weight percent.

TABLE 3

| Crush Strength Enhancement with Addition of Carbon |       |        |          |      |          |
|----------------------------------------------------|-------|--------|----------|------|----------|
| % HACN                                             | % CTN | % Guar | % Carbon | Form | Strength |
| 65.00                                              | 30.00 | 5.00   | 0.00     | EP   | 2.7 kg   |
| 64.75                                              | 30.00 | 4.50   | 0.75     | EP   | 5.7 kg   |
| 78.00                                              | 19.00 | 3.00   | 0.00     | pps. | 2.3 kg   |
| 72.90                                              | 23.50 | 3.00   | 0.60     | pps. | 5.8 kg   |
| 78.00                                              | 19.00 | 3.00   | 0.00     | EP   | 2.3 kg   |
| 73.00                                              | 23.50 | 3.00   | 0.50     | EP   | 4.1 kg   |

HACN = hexaamminecobalt(III) nitrate,  $[(\text{NH}_3)_6\text{Co}](\text{NO}_3)_3$  (Thiokol)CTN = copper(II) trihydroxy nitrate,  $[\text{Cu}_2(\text{OH}_3)\text{NO}_3]$  (Thiokol)

Guar = guar gum (Aldrich)

Carbon = "Monarch 1100" carbon black (Cabot)

EP = extruded pellet (see Example 22)

pps. = parallelepipeds (see Example 13)

strength = crush strength of pps. or extruded pellets in kilograms.

## Example 25

Hexaamminecobalt(III) nitrate was pressed into four gram pellets with a diameter of 0.5-inch. One half of the pellets were weighed and placed in a 95° C. oven for 700 hours. After aging, the pellets were weighed once again. No loss in weight was observed. The burn rate of the pellets held at ambient temperature was 0.16 ips at 1000 psi with a pressure exponent of 0.60. The burn rate of the pellets held at 95-C for 700 hours was 0.15 at 1000 psi with a pressure exponent of 0.68.

## Example 26

A gas-generating composition was prepared utilizing hexaamminecobalt(III) nitrate powder (76.00%, 273.6 g), copper(II) trihydroxy nitrate powder (16.00%, 57.69), 26 micron potassium nitrate (5.00%, 18.00 g), and guar gum (3.00%, 10.8 g). Deionized water (24.9% of the dry weight of the formulation, 16.2 g) was added to 65 g of the mixture which was blended for an additional five minutes on the Spex mixer/mill. This resulted in material with a dough-like consistency, which was processed into parallelepipeds (pps.) as in Example 13. The same process was repeated for the other 50–65 g batches of dry-blended generant and all the batches of pps. were blended together. The average dimensions of the pps. were 0.065 inch×0.074 inch×0.082 inch. Standard deviations on each of the dimensions were on the order of 0.005 inch. The average weight of the pps. was 7.42 mg. The bulk density, density as determined by dimensional measurements, and density as determined by solvent displacement were determined to be 0.86 g/cc, 1.15 g/cc, and 1.68 g/cc, respectively. Crush strengths of 2.1 kg (on the narrowest edge) were measured with a standard deviation of 0.3 kg. Some of the pps. were pressed into ten 0.5-inch diameter pellets weighing approximately three grams. Approximately 60 g of pps. and five 0.5-inch diameter pellets were placed in an oven held at 107° C. After 450 hours at this temperature, 0.25% and 0.41% weight losses were observed for the pps. and pellets, respectively. The remainder of the pps. and pellets were stored under ambient conditions. Burn rate data were obtained from both sets of pellets and are summarized in Table 4.

TABLE 4

| Burn Rate Comparison Before and After Accelerated Aging |                       |      |                   |
|---------------------------------------------------------|-----------------------|------|-------------------|
| Storage Conditions                                      | Burn Rate at 1000 psi |      | Pressure Exponent |
| 24–48 Hours @ Ambient                                   | 0.15 ips              | 0.72 |                   |
| 450 Hours @ 107° C.                                     | 0.15 ips              | 0.70 |                   |

## Example 27

Two simulators were constructed according to Example 4. In each igniter chamber, a blended mixture of 1.5 g of a stoichiometric blend of Mg/Sr(NO<sub>3</sub>)<sub>2</sub>/nylon and 1.5 grams of slightly over-oxidized B/KNO<sub>3</sub> igniter granules were placed. The diameter of the ports exiting the outer combustion chamber wall in each simulator were 0.177 inch. Thirty grams of ambient aged generant described in Example 26 in the form of parallelepipeds were secured in the combustion chamber of one simulator, whereas thirty grams of generant pps. aged at 107° C. were placed in the other combustion chamber. The simulators were attached to the 60-L tank described in Example 4. Test fire results are summarized in Table 5 below.

TABLE 5

| Aging Temp. | Test-Fire Results for Aged Generant |                    |                   |                             |                |                             |                  |
|-------------|-------------------------------------|--------------------|-------------------|-----------------------------|----------------|-----------------------------|------------------|
|             | Comb. Press. (psia)                 | Tank Press. (psia) | Tank Temp. (° K.) | NH <sub>3</sub> Level (ppm) | CO Level (ppm) | NO <sub>x</sub> Level (ppm) | Part. Level (mg) |
| Amb.        | 2171                                | 31.9               | 628               | 350                         | 500            | 80                          | 520              |
| 107° C.     | 2080                                | 31.6               | 629               | 160                         | 500            | 100                         | 480              |

## Example 28

A mixture of 2Co(NH<sub>3</sub>)<sub>3</sub>(NO<sub>2</sub>)<sub>3</sub> and Co(NH<sub>3</sub>)<sub>4</sub>(NO<sub>2</sub>)<sub>2</sub> Co(NH<sub>3</sub>)<sub>2</sub>(NO<sub>2</sub>)<sub>4</sub> was prepared and pressed in a pellet having a diameter of approximately 0.504 inch. The complexes were prepared within the scope of the teachings of the Hagel, et al. reference identified above. The pellet was placed in a test bomb, which was pressurized to 1,000 psi with nitrogen gas.

The pellet was ignited with a hot wire and burn rate was measured and observed to be 0.38 inch per second. Theoretical calculations indicated a flame temperature of 1805° C. From theoretical calculations, it was predicted that the major reaction products would be solid CoO and gaseous reaction products. The major gaseous reaction products were predicted to be as follows:

| Product          | Volume % |
|------------------|----------|
| H <sub>2</sub> O | 57.9     |
| N <sub>2</sub>   | 38.6     |
| O <sub>2</sub>   | 3.1      |

## Example 29

A quantity of Co(NH<sub>3</sub>)<sub>2</sub>(NO<sub>2</sub>)<sub>4</sub> was prepared according to the teachings of Example 1 and tested using differential scanning calorimetry. It was observed that the complex produced a vigorous exotherm at 200° C.

Theoretical calculations were undertaken for  $\text{Co}(\text{NH}_3)_3(\text{NO}_2)_3$ . Those calculations indicated a flame temperature of about 2,000° K and a gas yield of about 1.75 times that of a conventional sodium azide gas-generating compositions based on equal volume of generating composition ("performance ratio"). Theoretical calculations were also undertaken for a series of gas-generating compositions. The composition and the theoretical performance data is set forth below in Table 6.

TABLE 6

| Gas Generant                                                                  | Ratio | Temp. (C.) | Perf. Ratio |
|-------------------------------------------------------------------------------|-------|------------|-------------|
| $\text{Co}(\text{NH}_3)_3(\text{NO}_2)_3$                                     | —     | 1805       | 1.74        |
| $\text{NH}_4[\text{Co}(\text{NH}_3)_2(\text{NO}_2)_4]$                        | —     | 1381       | 1.81        |
| $\text{NH}_4[\text{Co}(\text{NH}_3)_2(\text{NO}_2)_4]/\text{B}$               | 99/1  | 1634       | 1.72        |
| $\text{Co}(\text{NH}_3)_6(\text{NO}_3)_3$                                     | —     | 1585       | 2.19        |
| $[\text{Co}(\text{NH}_3)_5(\text{NO}_3)][\text{NO}_3]_2$                      | —     | 1637       | 2.00        |
| $[\text{Fe}(\text{N}_2\text{H}_4)_4][\text{NO}_3]_2/\text{Sr}(\text{NO}_3)_2$ | 87/13 | 2345       | 1.69        |
| $[\text{Co}(\text{NH}_3)_6](\text{ClO}_4)_3/\text{CaH}_2$                     | 86/14 | 2577       | 1.29        |
| $[\text{Co}(\text{NH}_3)_5(\text{NO}_2)][\text{NO}_3]_2$                      | —     | 1659       | 2.06        |

Performance ratio is a normalized relation to a unit volume of azide-based gas generant. The theoretical gas yield for a typical sodium azide-based gas generant (68 wt. %  $\text{NaN}_3$ ; 30 wt % of  $\text{MoS}_2$ ; 2 wt % of S) is about 0.85 g gas/cc  $\text{NaN}_3$  generant.

Example 31

Theoretical calculations were conducted on the reaction of  $[\text{Co}(\text{NH}_3)_6](\text{ClO}_4)_3$  and  $\text{CaH}_2$  as listed in Table 6 to evaluate its use in a hybrid gas generator. If this formulation is allowed to undergo combustion in the presence of 6.80 times its weight in argon gas, the flame temperature decreases from 2577° C. to 1085° C., assuming 100% efficient heat transfer. The output gases consist of 86.8% by volume argon, 1600 ppm by volume hydrogen chloride, 10.2% by volume water, and 2.9% by volume nitrogen. The total slag weight would be 6.1% by mass.

Example 32

Pentaamminecobalt(III) nitrate complexes were synthesized, which contain a common ligand in addition to  $\text{NH}_3$ . Aquopentaamminecobalt (III) nitrate and pentaamminecarbonatocobalt (III) nitrate were synthesized according to *Inora. Svn.*, vol. 4, p. 171 (1973). Pentaamminehydroxocobalt(III) nitrate was synthesized according to H. J. S. King, *J. Chem. Soc.*, p. 2105 (1925) and O. Schmitz, et al., *Zeit. Anorg. Chem.*, vol. 300, p. 186 (1959). Three lots of gas generant were prepared utilizing the pentaamminecobalt(III) nitrate complexes described above. In all cases guar gum was added as a binder. Copper(II) trihydroxy nitrate,  $[\text{Cu}_2(\text{OH})_3\text{NO}_3]$ , was added as the co-oxidizer where needed. Burn rates were determined from 0.5-inch diameter burn rate pellets. The results are summarized below in Table 7.

TABLE 7

| Formulations Containing $[\text{Co}(\text{NH}_3)_5\text{X}](\text{NO}_3)_2$      |                              |                         |
|----------------------------------------------------------------------------------|------------------------------|-------------------------|
| Formulation                                                                      | % $\text{H}_2\text{O}$ Added | Burn Rate               |
| 97.0% $[\text{Co}(\text{NH}_3)_5(\text{H}_2\text{O})](\text{NO}_3)_3$<br>3% guar | 27%                          | 0.16 ips<br>at 1000 psi |

TABLE 7-continued

| Formulations Containing $[\text{Co}(\text{NH}_3)_5\text{X}](\text{NO}_3)_2$ |                              |                         |
|-----------------------------------------------------------------------------|------------------------------|-------------------------|
| Formulation                                                                 | % $\text{H}_2\text{O}$ Added | Burn Rate               |
| 68.8% $[\text{Co}(\text{NH}_3)_5(\text{OH})](\text{NO}_3)_2$                | 55%                          | 0.14 ips<br>at 1000 psi |
| 28.2% $[\text{Cu}_2(\text{OH})_3\text{NO}_3]$<br>3.0% guar                  |                              |                         |
| 48.5% $[\text{Co}(\text{NH}_3)_5(\text{CO}_3)](\text{NO}_3)_2$              | 24%                          | 0.06 ips<br>at 4150 psi |
| 48.5% $[\text{Cu}_2(\text{OH})_3\text{NO}_3]$<br>3.0% guar                  |                              |                         |

## SUMMARY

In summary the present invention provides gas-generating materials that overcome some of the limitations of conventional al azide-based gas-generating compositions. The complexes of the present invention produce nontoxic gaseous products including water vapor, oxygen, and nitrogen. Certain of the complexes are also capable of efficient decomposition to a metal or metal oxide, and nitrogen and water vapor. Finally, reaction temperatures and burn rates are within acceptable ranges.

The invention may be embodied in other specific forms without departing from its essential characteristics. The described embodiments are to be considered in all respects only as illustrative and not restrictive. The scope of the invention is, therefore, indicated by the appended claims rather than by the foregoing description.

What is claimed is:

1. A solid gas-generating composition formulated for generating gas suitable for use in deploying an air bag or balloon from a supplemental restraint system, the solid gas-generating composition consisting essentially of:  
at least one complex of a metal cation and at least one neutral ligand which comprises ammonia, wherein the metal cation is a transition metal cation or an alkaline earth metal cation, and sufficient anion to balance a charge of the metal cation;  
and calcium stearate; and  
optionally co-oxidizer in an amount less than 50% by weight of the solid gas-generating composition.
2. A solid gas-generating composition formulated for generating gas suitable for use in deploying an air bag or balloon from a supplemental restraint system, the solid gas-generating composition consisting essentially of:  
a complex of a metal cation and a neutral ligand containing hydrogen and nitrogen and sufficient oxidizing anion to balance a charge of the metal cation, wherein the complex is selected from the group consisting of metal nitrite ammines, metal nitrate ammines, metal perchlorate ammines, and mixtures thereof; and  
a release agent.
3. The solid gas-generating composition as defined in claim 2, wherein the metal cation is a transition metal, alkaline earth metal, metalloid, or lanthanide metal cation.
4. The solid gas-generating composition as defined in claim 3, wherein the transition metal cation is a cobalt cation.
5. The solid gas-generating composition as defined in claim 3, wherein the metal cation is a cation of a metal selected from the group consisting of cobalt, magnesium, manganese, nickel, titanium, copper, chromium, zinc, tin, rhodium, iridium, ruthenium, palladium and platinum.
6. The solid gas-generating composition as defined in claim 2, wherein the oxidizing anion is selected from the

23

group consisting of nitrate, nitrite, chlorate, perchlorate, peroxide, and superoxide.

7. The solid gas-generating composition as defined in claim 2, wherein the oxidizing anion is free of carbon.

8. The gas-generating composition as defined in claim 2, further comprising a binder.

9. The solid gas-generating composition as defined in claim 8, (wherein the binder is water soluble).

10. The solid gas-generating composition as defined in claim 9, wherein the binder is selected from naturally occurring gums, polyacrylic acids, and polyacrylamides.

11. The solid gas-generating composition as defined in claim 8, wherein the binder is not water soluble.

12. The solid gas-generating composition as defined in claim 8, wherein the binder is selected from nitrocellulose, VAAR (vinyl acetate vinyl alcohol resin), and nylon.

13. The solid gas-generating composition as defined in claim 2, wherein the complex is hexamminecobalt (II) nitrate  $[(\text{NH}_3)_6\text{Co}](\text{NO}_3)_3$  and the composition further includes copper (II) trihydroxy nitrate  $(\text{Cu}_2(\text{OH})_3\text{NO}_3)$ .

14. The solid gas-generating composition as defined in claim 2, wherein the complex includes at least one common ligand, in addition to the ammonia ligand.

15. The solid gas-generating composition as defined in claim 14, wherein the common ligand is selected from the group consisting of aquo ( $\text{H}_2\text{O}$ ), hydroxo ( $\text{OH}$ ), perhydroxo ( $\text{O}_2\text{H}$ ), peroxy ( $\text{O}_2$ ), carbonato ( $\text{CO}_3$ ), carbonyl ( $\text{CO}$ ), oxalato ( $\text{C}_2\text{O}_4$ ), nitrosyl ( $\text{NO}$ ), cyano ( $\text{CN}$ ), isocyanato ( $\text{NC}$ ), isothiocyanato ( $\text{NCS}$ ), thiocyanato ( $\text{SCN}$ ), amido ( $\text{NH}_2$ ), imido ( $\text{NH}$ ), sulfate ( $\text{SO}_4$ ), chloro ( $\text{Cl}$ ), fluoro ( $\text{F}$ ), phosphate ( $\text{PO}_4$ ), and ethylenediaminetetraacetic acid (EDTA) ligands.

16. The solid gas-generating composition as defined in claim 2, wherein the complex includes a common counter ion in addition to the oxidizing anion.

17. The solid gas-generating composition as defined in claim 16, wherein the common counter ion is selected from the group consisting of hydroxide ( $\text{OH}^-$ ), chloride ( $\text{Cl}^-$ ), fluoride ( $\text{F}^-$ ), cyanide ( $\text{CN}^-$ ), thiocyanate ( $\text{SCN}^-$ ), carbonate ( $\text{CO}_3^{2-}$ ), sulfate ( $\text{SO}_4^{2-}$ ), phosphate ( $\text{PO}_4^{3-}$ ), oxalate ( $\text{C}_2\text{O}_4^{2-}$ ), borate ( $\text{B}_4^{5-}$ ), and ammonium ( $\text{NH}_4^+$ ) counter ions.

18. The solid gas-generating composition as defined in claim 2, wherein the composition is formulated from ingredients comprising:

at least one complex of

a metal cation

at least one ammonia ligand, and

sufficient oxidizing anion to balance a charge of the complex wherein the composition contains about 50% to about 80% by weight of the complex; and

the release agent.

19. The solid gas-generating composition as defined in claim 2, further comprising a co-oxidizer.

20. The solid gas-generating composition as defined in claim 19, wherein the co-oxidizer is selected from the group consisting of alkali, alkaline earth, lanthanide or ammonium perchlorates, chlorates, peroxides, nitrites, and nitrates.

21. The solid gas-generating composition as defined in claim 19, (wherein the co-oxidizer is selected from the group consisting of metal oxides, metal hydroxides, metal peroxides, metal oxide hydrates, metal oxide hydroxides, metal hydrous oxides, basic metal carbonates, basic metal nitrates, and mixtures thereof.

22. The solid gas-generating composition as defined in claim 19, wherein the co-oxidizer is selected from the group consisting of oxides of copper, cobalt, manganese, tungsten bismuth, molybdenum, and iron.

24

23. The solid gas-generating composition as defined in claim 19, wherein the co-oxidizer is a metal oxide selected from the group consisting of  $\text{CuO}$ ,  $\text{CO}_2\text{O}_3$ ,  $\text{CO}_3\text{O}_4$ ,  $\text{CoFe}_2\text{O}_4$ ,  $\text{Fe}_2\text{O}_3$ ,  $\text{MoO}_3$ ,  $\text{Bi}_2\text{MoO}_6$ , and  $\text{Bi}_2\text{O}_3$ .

24. The solid gas-generating composition as defined in claim 19, wherein the co-oxidizer is a metal hydroxide selected from the group consisting of  $\text{Fe}(\text{OH})_3$ ,  $\text{Co}(\text{OH})_3$ ,  $\text{Co}(\text{OH})_2$ ,  $\text{Ni}(\text{OH})_2$ ,  $\text{Cu}(\text{OH})_2$ , and  $\text{Zn}(\text{OH})_2$ .

25. The solid gas-generating composition as defined in claim 19, wherein the co-oxidizer is a metal oxide hydrate or metal hydrous oxide selected from the group consisting of  $\text{Fe}_2\text{O}_3 \cdot \text{xH}_2\text{O}$ ,  $\text{SnO}_2 \cdot \text{xH}_2\text{O}$ , and  $\text{MoO}_3 \cdot \text{H}_2\text{O}$ .

26. The solid gas-generating composition as defined in claim 19, wherein the co-oxidizer is a metal oxide hydroxide selected from the group consisting of  $\text{CoO}(\text{OH})_2$ ,  $\text{FeO}(\text{OH})_2$ ,  $\text{FeO}(\text{OH})_2$ ,  $\text{MnO}(\text{OH})_2$ , and  $\text{MnO}(\text{OH})_3$ .

27. The solid gas-generating composition as defined in claim 19, wherein the co-oxidizer is a basic metal carbonate selected from the group consisting of  $\text{CuCO}_3$ ,  $\text{Cu}(\text{OH})_2$  (malachite),  $2\text{Co}(\text{CO}_3) \cdot 3\text{Co}(\text{OH})_7\text{H}_2\text{O}$ ,  $\text{Co}_{0.69}\text{Fe}_{0.34}(\text{CO}_3)_{0.7}(\text{OH})_2$ ,  $\text{Na}_3[\text{Co}(\text{CO}_3)_3]3\text{H}_2\text{O}$ ,  $\text{Zl}_2(\text{C}_3)(\text{OH})_2$ ,  $\text{Bi}_2\text{Mg}(\text{CO}_3)_2(\text{OH})_4$ ,

$\text{Fe}(\text{CO}_3)_{0.12}(\text{OH})_{2.76}\text{Cu}_{1.54}\text{Zn}_{0.46}(\text{CO}_3)(\text{OH})_2$ ,  $\text{CO}_{0.49}\text{Cu}_{0.51}(\text{CO}_3)_{0.43}(\text{OH})_{1.1}\text{Ti}_3\text{Bi}_4(\text{CO}_3)_2(\text{OH})_2\text{O}_9(\text{H}_2\text{O})_2$ , and  $(\text{BiO})_2\text{CO}_3$ .

28. The solid gas-generating composition as defined in claim 19, wherein the co-oxidizer is a basic metal nitrate selected from the group consisting of  $\text{Cu}_2(\text{OH})_3\text{NO}_3\text{CO}_2(\text{OH})_3\text{NO}_3$ ,  $\text{CuCo}(\text{OH})_2\text{NO}_3$ ,  $\text{Zn}_2(\text{OH})_3\text{NO}_3$ ,  $\text{Mn}(\text{OH})_2\text{NO}_3$ ,  $\text{Fe}_4(\text{OH})_{11}\text{NO}_3 \cdot 2\text{H}_2\text{O}$ ,  $\text{Mo}(\text{NO}_3)_2\text{O}_2$ ,  $\text{BiONO}_3 \cdot \text{H}_2\text{O}$ , and  $\text{Ce}(\text{OH})(\text{NO}_3)_3 \cdot 3\text{H}_2\text{O}$ .

29. The solid gas-generating composition as defined in claim 2, further comprising a carbon powder present from 0.1% to 6% by weight of the solid gas-generating composition.

30. The solid gas-generating composition as defined in claim 2, wherein the complex is selected from the group consisting of metal nitrate ammines.

31. The solid gas-generating composition as defined in claim 30, wherein the release agent comprises graphite, molybdenum sulfide, calcium stearate or boron nitride.

32. A solid gas-generating composition formulated for generating gas suitable for use in deploying an air bag or balloon from a supplemental restraint system, the solid gas-generating composition consisting essentially of:

a complex of a metal cation and a neutral ligand containing hydrogen and nitrogen and sufficient oxidizing anion to balance the charge of the metal cation, wherein the complex is selected from the group consisting of metal nitrite ammines, metal nitrate ammines, metal perchlorate ammines, and mixtures thereof; wherein the composition contains from 48.5% to less than 100% of the complex, and the composition contains a release agent.

33. The solid gas-generating composition according to claim 2, wherein when the composition combusts, the combustion takes place at a rate and a temperature sufficient to qualify the composition for use as a gas-generating composition to generate gas suitable for use in deploying the air bag or the balloon.